# EUROPEAN PATENT SPECIFICATION

(11) **EP 2 738 613 B1**
(45) Date of publication and mention of the grant of the patent: **03.02.2016**
(21) Application number: 13193400.2
(22) Date of filing: 19.11.2013
(51) Int. Cl.: G03G 5/07, G03G 5/147, G03G 5/05

(54) **Electrophotographic photosensitive member, method for producing electrophotographic photosensitive member, process cartridge and electrophotographic apparatus**
Elektrofotografisches lichtempfindliches Element, Verfahren zur Herstellung des elektrofotografischen lichtempfindlichen Elements, Prozesskartusche und elektrofotografische Vorrichtung
Élément photosensible électrophotographique, procédé de fabrication d'un élément photosensible électrophotographique, cartouche de traitement et appareil électrophotographique

(30) Priority: 30.11.2012 JP 2012263258; 29.10.2013 JP 2013224419
(43) Date of publication of application: 04.06.2014
(73) Proprietor: Canon Kabushiki Kaisha, Tokyo 146-8501 (JP)
(72) Inventor: Maruyama, Akihiro, Tokyo,, Tokyo 146-8501 (JP); Ogaki, Harunobu, Tokyo,, Tokyo 146-8501 (JP); Yamamoto, Yuki, Tokyo,, Tokyo 146-8501 (JP)
(74) Representative: TBK

(56) References cited:
- EP-A1- 2 042 931
- EP-A1- 2 278 407
- WO-A1-2012/141016

## Description

### BACKGROUND OF THE INVENTION

### Field of the Invention

The present invention relates to an electrophotographic photosensitive member, and a process cartridge and an electrophotographic apparatus including the electrophotographic photosensitive member.

### Description of the Related Art

As an electrophotographic photosensitive member included in an electrophotographic apparatus, electrophotographic photosensitive members containing organic photoconductive substances have been earnestly developed. An electrophotographic photosensitive member generally contains a support and a photosensitive layer formed on the support and containing an organic photoconductive substance. Furthermore, the photosensitive layer is generally of a laminated type (a successive layer type) containing a charge-generating layer and a charge-transporting layer stacked in this order on the support.

In electrophotographic process, the surface of an electrophotographic photosensitive member is brought into contact with various materials including a developer, a charging member, a cleaning blade, paper and a transferring member (which are hereinafter sometimes generically designated as "contact members"). Therefore, one of characteristics required of an electrophotographic photosensitive member is reduction of image degradation derived from contact stress caused by these contact members. In particular, in accordance with recent improvement in the durability of an electrophotographic photosensitive member, further improvement is demanded in persistence of the effect of reducing image degradation derived from the contact stress and suppression of potential variation in repeated use.

With respect to persistent relaxation of the contact stress and suppression of potential variation in repeated use of an electrophotographic photosensitive member, International Publication No. WO2010/008095 proposes a method for forming a matrix-domain structure in a surface layer by using a siloxane resin in which a siloxane structure is incorporated into a molecular chain. This publication describes that the persistent relaxation of the contact stress and the suppression of potential variation in repeated use of an electrophotographic photosensitive member can be both attained by using a polyester resin having a specific siloxane structure incorporated thereinto.

Although the electrophotographic photosensitive member disclosed in International Publication No. WO2010/008095 attains both of the persistent relaxation of the contact stress and the suppression of potential variation in repeated use, further improvement is demanded in order to realize an electrophotographic apparatus operable at a higher speed and capable of producing a larger number of printed copies. As a result of study made by the present inventors, it has been revealed that further improvement can be achieved by allowing an electrophotographic photosensitive member to contain a specific compound in forming a matrix-domain structure.

### SUMMARY OF THE INVENTION

An object of the present invention is to provide an electrophotographic photosensitive member and a method for producing the same in which persistent relaxation of contact stress and suppression of potential variation in repeated use of an electrophotographic photosensitive member are both achieved at a high level. Another object is to provide a process cartridge and an electrophotographic apparatus including the electrophotographic photosensitive member.

The present invention relates to an electrophotographic photosensitive member including: a support; a charge-generating layer formed on the support; and a charge-transporting layer formed on the charge-generating layer, in which the charge-transporting layer is a surface layer of the electrophotographic photosensitive member, and the charge-transporting layer has a matrix-domain structure having: a domain which includes a compound D having a structural unit represented by the following formula (O-1) and a structural unit represented by the following formula (0-2); and at least one resin selected from the group consisting of a resin A1 having a structural unit represented by the following formula (A-1) and a structural unit represented by the following formula (B), and a resin A2 having a structural unit represented by the following formula (A-2) and a structural unit represented by the following formula (B); and a matrix which includes a resin C having a structural unit represented by the following formula (C) and a charge-transporting substance, and a content of the structural unit represented by the formula (A-1) and the structural unit represented by the formula (A-2) is from 10% by mass to 40% by mass based on the total mass of the resin A1 and the resin A2: where, m¹¹ represents 0 or 1, X¹¹ represents an ortho-phenylene group, a meta-phenylene group, a para-phenylene group, a bivalent group having two para-phenylene groups bonded with a methylene group, or a bivalent group having two para-phenylene groups bonded with an oxygen atom, Z¹¹ and Z¹² each independently represents an alkylene group having 1 to 4 carbon atoms, R¹¹ to R¹⁴ each independently represents an alkyl group having 1 to 4 carbon atoms, or a phenyl group, n¹¹ represents the repetition number of a structure within brackets, and an average of n¹¹ in the resin A1 ranges from 20 to 150, where, m²¹ represents 0 or 1, X²¹ represents an ortho-phenylene group, a meta-phenylene group, a para-phenylene group, a bivalent group having two para-phenylene groups bonded with a methylene group, or a bivalent group having two para-phenylene groups bonded with an oxygen atom, Z²¹ to Z²³ each independently represents an alkylene group having 1 to 4 carbon atoms, R¹⁶ to R²⁷ each independently represents an alkyl group having 1 to 4 carbon atoms, or a phenyl group, n²¹, n²² and n²³ each independently represents the repetition number of a structure within brackets, an average of n²¹ in the resin A2 ranges from 1 to 10, an average of n²² in the resin A2 ranges from 1 to 10, and an average of n²³ in the resin A2 ranges from 20 to 200, where, m³¹ represents 0 or 1, X³¹ represents an ortho-phenylene group, a meta-phenylene group, a para-phenylene group, a bivalent group having two para-phenylene groups bonded with a methylene group, or a bivalent group having two para-phenylene groups bonded with an oxygen atom, Y³¹ represents a single bond, a methylene group, an ethylidene group, a propylidene group, a cyclohexylidene group, a phenylmethylene group, a phenylethylidene group or an oxygen atom, and R³¹ to R³⁸ each independently represents a hydrogen atom or a methyl group, where, m⁴¹ represents 0 or 1, X⁴¹ represents an ortho-phenylene group, a meta-phenylene group, a para-phenylene group, a bivalent group having two para-phenylene groups bonded with a methylene group, or a bivalent group having two para-phenylene groups bonded with an oxygen atom, Y⁴¹ represents a single bond, a methylene group, an ethylidene group, a propylidene group, a cyclohexylidene group, a phenylmethylene group, a phenylethylidene group or an oxygen atom, and R⁴¹ to R⁴⁸ each independently represents a hydrogen atom or a methyl group, where, R⁶¹ represents a hydrogen atom or a methyl group, R⁶² represents a phenyl group, a cyano group, a carbamoyl group, or a group represented by the formula - COOR⁶⁴, where R⁶⁴ represents a hydrogen atom, a methyl group, an ethyl group, a propyl group, an isopropyl group, a butyl group, an isobutyl group, a 2-ethylhexyl group, a nonyl group, an isononyl group, a cyclohexyl group, a 2-methoxyethyl group or a 2-hydroxyethyl group,
R⁶³ represents a hydrogen atom or a methyl group, n⁶¹ represents the repetition number of a structure within brackets, and an average of n⁶¹ in the compound D ranges from 1 to 500.

Furthermore, the present invention relates to a process cartridge detachably attachable to a main body of an electrophotographic apparatus, the process cartridge integrally supports, the electrophotographic photosensitive member, and at least one device selected from the group consisting of a charging device, a developing device, a transferring device and a cleaning device.

Moreover, the present invention relates to an electrophotographic apparatus including the electrophotographic photosensitive member, a charging device, an exposing device, a developing device and a transferring device.

According to the present invention, an excellent electrophotographic photosensitive member and a method for producing the same in which persistent relaxation of contact stress and suppression of potential variation in repeated use of an electrophotographic photosensitive member are both attained at a high level can be provided. Besides, a process cartridge and an electrophotographic apparatus including the electrophotographic photosensitive member can be provided.

Further features of the present invention will become apparent from the following description of exemplary embodiments with reference to the attached drawings.

### BRIEF DESCRIPTION OF THE DRAWINGS

FIG. 1 is a diagram illustrating an example of the schematic structure of an electrophotographic apparatus provided with a process cartridge including an electrophotographic photosensitive member.
FIGS. 2A and 2B are diagrams illustrating examples of a layered structure of an electrophotographic photosensitive member.

### DESCRIPTION OF THE EMBODIMENTS

Preferred embodiments of the present invention will now be described in detail in accordance with the accompanying drawings.

According to the present invention, a charge-transporting layer of an electrophotographic photosensitive member has a matrix-domain structure including the following matrix and the following domain.

The domain includes a compound D having a structural unit represented by the following formula (O-1) and a structural unit represented by the following formula (0-2). The domain further includes at least one resin selected from the group consisting of: a resin A1 having a structural unit represented by the following formula (A-1) and a structural unit represented by the following formula (B); and a resin A2 having a structural unit represented by the following formula (A-2) and a structural unit represented by the following formula (B).

The matrix includes a resin C having a structural unit represented by the following formula (C), and a charge-transporting substance.

The content of the structural unit represented by the formula (A-1) and the structural unit represented by the formula (A-2) is from 10% by mass to 40% by mass based on the total mass of the resin A1 and the resin A2.

In the formula (A-1), m¹¹ represents 0 or 1; X¹¹ represents an ortho-phenylene group, a meta-phenylene group, a para-phenylene group, a bivalent group having two para-phenylene groups bonded with a methylene group, or a bivalent group having two para-phenylene groups bonded with an oxygen atom; Z¹¹ and Z¹² each independently represents an alkylene group having 1 to 4 carbon atoms; R¹¹ to R¹⁴ each independently represents an alkyl group having 1 to 4 carbon atoms, or a phenyl group; n¹¹ represents the repetition number of a structure within brackets, and an average of n¹¹ in the resin A1 ranges from 20 to 150.

In the formula (A-2), m²¹ represents 0 or 1; X²¹ represents an ortho-phenylene group, a meta-phenylene group, a para-phenylene group, a bivalent group having two para-phenylene groups bonded with a methylene group, or a bivalent group having two para-phenylene groups bonded with an oxygen atom; Z²¹ to Z²³ each independently represents an alkylene group having 1 to 4 carbon atoms; R¹⁶ to R²⁷ each independently represents an alkyl group having 1 to 4 carbon atoms, or a phenyl group; n²¹, n²² and n²³ each independently represents the repetition number of a structure within brackets, an average of n²¹ in the resin A2 ranges from 1 to 10, an average of n²² in the resin A2 ranges from 1 to 10, and an average of n²³ in the resin A2 ranges from 20 to 200.

In the formula (B), m³¹ represents 0 or 1; X³¹ represents an ortho-phenylene group, a meta-phenylene group, a para-phenylene group, a bivalent group having two para-phenylene groups bonded with a methylene group, or a bivalent group having two para-phenylene groups bonded with an oxygen atom; Y³¹ represents a single bond, a methylene group, an ethylidene group, a propylidene group, a cyclohexylidene group, a phenylmethylene group, a phenylethylidene group or an oxygen atom; and R³¹ to R³⁸ each independently represents a hydrogen atom or a methyl group.

In the formula (C), m⁴¹ represents 0 or 1; X⁴¹ represents an ortho-phenylene group, a meta-phenylene group, a para-phenylene group, a bivalent group having two para-phenylene groups bonded with a methylene group, or a bivalent group having two para-phenylene groups bonded with an oxygen atom; Y⁴¹ represents a single bond, a methylene group, an ethylidene group, a propylidene group, a cyclohexylidene group, a phenylmethylene group, a phenylethylidene group or an oxygen atom; and R⁴¹ to R⁴⁸ each independently represents a hydrogen atom or a methyl group.

In the structural unit represented by either of the formulas (B) and (C), the propylidene group can be a 2,2-propylidene group, and the phenylethylidene group can be a 1-phenyl-1,1-ethylidene group.

In the formula (O-1), R⁶¹ represents a hydrogen atom or a methyl group; R⁶² represents a phenyl group, a cyano group, a carbamoyl group, or a group represented by the formula -COOR⁶⁴, where R⁶⁴ represents a hydrogen atom, a methyl group, an ethyl group, a propyl group, an isopropyl group, a butyl group, an isobutyl group, a 2-ethylhexyl group, a nonyl group, an isononyl group, a cyclohexyl group, a 2-methoxyethyl group or a 2-hydroxyethyl group.

In the formula (0-2), R⁶³ represents a hydrogen atom or a methyl group; n⁶¹ represents the repetition number of a structure within brackets; and an average of n⁶¹ in the compound D ranges from 1 to 500.

Since the compound D has the structural units represented by the formulas (O-1) and (0-2), the compound D is contained in the domain containing the resin A1 and the resin A2. Particularly in the formula (O-1), the substituent of R⁶² functions as an anchor unit so as to increase affinity with structures of the resin A1 and the resin A2 other than a Si portion, which probably causes the compound D to be easily entangled with molecular chains of the resin A1 and the resin A2. This seems to be the reason why the compound D is contained in the domain containing the resin A1 and the resin A2.

The charge-transporting layer of the present invention has the matrix-domain structure including a matrix containing the charge-transporting substance and the resin C, and domains formed in the matrix and containing the resin A1, the resin A2 and the compound D. When the matrix-domain structure is compared to a "sea-island structure," the matrix corresponds to a sea part and the domain corresponds to an island part.

Each domain containing the resin A1, the resin A2 and the compound D has a granular (island) structure formed in the matrix containing the charge-transporting substance and the resin C. The domains each containing the resin A1, the resin A2 and the compound D are respectively spaced from one another to be independently present in the matrix. Such a matrix-domain structure can be verified by observing a surface of the charge-transporting layer or a cross-section of the charge-transporting layer.

The observation of the state of the matrix-domain structure or measurement of the domains can be performed by using, for example, a commercially available laser microscope, optical microscope, electron microscope or atomic force microscope. Any of these microscopes may be used with prescribed magnification for observing the state of the matrix-domain structure or measuring the structure of each domain.

The number average particle size of the domains can be from 100 nm to 3,000 nm. Furthermore, the size distribution of the particle sizes of the respective domains can be smaller from the viewpoint of uniformity in a coating film and a stress relaxation effect. For calculating the number average particle size, arbitrary 100 domains are selected from domains observed with a microscope in a vertical cross-section of the charge-transporting layer. The maximum diameters of the selected domains are measured, and the maximum diameters of the domains are averaged for calculating the number average particle size. Incidentally, when a cross-section of the charge-transporting layer is observed with a microscope, image information along the depth direction can be obtained, so as to acquire a three-dimensional image of the charge-transporting layer.

The matrix-domain structure of the charge-transporting layer can be formed as follows: A charge-transporting layer coating solution containing the charge-transporting substance, the resin A1, the resin A2, the compound D and the resin C is prepared for forming a coating film of the charge-transporting layer coating solution, and the coating film is dried, thereby forming the charge-transporting layer.

When the domains containing the resin A1, the resin A2 and the compound D are efficiently formed in the charge-transporting layer, persistent relaxation of the contact stress can be more effectively exhibited. Since the domains containing the resin A1, the resin A2 and the compound D are formed, localization of the compound D on an interface between the charge-transporting layer and the charge-generating layer can be suppressed, so that the potential variation occurring in repeated use of the electrophotographic photosensitive member can be suppressed. This is probably because a barrier to charge movement caused by localization of siloxane components on the interface between the charge-transporting layer and the charge-generating layer can be reduced, in the movement of charge from the charge-generating layer to the charge-transporting layer, by forming the aforementioned domains.

### (Resin A1 and Resin A2)

Next, the resin A1 and the resin A2 will be described.

The resin A1 has a structural unit represented by the formula (A-1) and a structural unit represented by the formula (B). The resin A2 has the structural unit represented by the formula (A-2) and a structural unit represented by the formula (B).

In the formula (A-1), X¹¹ may be a single group or two or more groups. Z¹¹ and Z¹² each represents an alkylene group having 1 to 4 carbon atoms, and specific examples include a methylene group, an ethylene group, a propylene group and a butylene group. From the viewpoint of the effect of relaxing the contact stress, Z¹¹ and Z¹² each can represent a propylene group. If R¹¹ to R¹⁴ each represents an alkyl group having 1 to 4 carbon atoms, specific examples include a methyl group, an ethyl group, a propyl group and a butyl group. From the viewpoint of the effect of relaxing the contact stress, R¹¹ to R¹⁴ each can represent a methyl group.

If the average of n¹¹ in the resin A1 ranges from 20 to 150, the domains containing the resin A1, the resin A2 and the compound D can be efficiently formed in the matrix containing the charge-transporting substance and the resin C. In particular, the average of n¹¹ can range from 40 to 80.

Examples of the structural unit represented by the formula (A-1) are shown in Table 1 below.

**(Table 1)**

| Formula (A-1) | m11 | X11 | R11-R14 | Z11, Z12 | n11 |
|---|---|---|---|---|---|
| A-1-1 | 1 | ortho-phenylene | methyl | propylene | 40 |
| A-1-2 | 1 | meta-phenylene | methyl | propylene | 40 |
| A-1-3 | 1 | para-phenylene | methyl | propylene | 40 |
| A-1-4 | 1 | | methyl | propylene | 40 |
| A-1-5 | 1 | | methyl | propylene | 40 |
| A-1-6 | 1 | ortho-phenylene | methyl | propylene | 80 |
| A-1-7 | 1 | meta-phenylene | methyl | propylene | 80 |
| A-1-8 | 1 | para-phenylene | methyl | propylene | 80 |
| A-1-9 | 1 | | ethyl | propylene | 80 |
| A-1-10 | 1 | | methyl | propylene | 80 |
| A-1-11 | 1 | ortho-phenylene | butyl | methylene | 100 |
| A-1-12 | 1 | meta-phenylene | phenyl | ethylene | 150 |
| A-1-13 | 1 | para-phenylene | methyl | butylene | 20 |
| A-1-14 | 1 | para-phenylene | propyl | butylene | 120 |
| A-1-15 | 0 | - | methyl | propylene | 40 |
| A-1-16 | 0 | - | ethyl | propylene | 80 |
| A-1-17 | 0 | - | methyl | propylene | 60 |
| A-1-18 | 0 | - | butyl | methylene | 100 |
| A-1-19 | 0 | - | phenyl | ethylene | 150 |
| A-1-20 | 0 | - | methyl | butylene | 20 |
| A-1-21 | 0 | - | propyl | butylene | 120 |

In the formula (A-2), X²¹ may be a single group or two or more groups. Z²¹ to Z²³ each represents an alkylene group having 1 to 4 carbon atoms, and specific examples include a methylene group, an ethylene group, a propylene group and a butylene group. From the viewpoint of the effect of relaxing the contact stress, Z²¹ and Z²² can each represent a propylene group and Z²³ can represent an ethylene group. If R¹⁶ to R²⁷ each represents an alkyl group having 1 to 4 carbon atoms, specific examples include a methyl group, an ethyl group, a propyl group and a butyl group. From the viewpoint of the effect of relaxing the contact stress, R¹⁶ to R²⁷ can each represent a methyl group.

The average of n²¹ in the resin A2 ranges from 1 to 10, the average of n²² in the resin A2 ranges from 1 to 10, and the average of n²³ in the resin A2 ranges from 20 to 200. If these averages are within these ranges, the domains containing the resin A1, the resin A2 and the compound D can be efficiently formed in the matrix containing the charge-transporting substance and the resin C. The averages of n²¹ and n²² can range from 1 to 5, and the average of n²³ can range from 40 to 120. Examples of the structural unit represented by the formula (A-2) are shown in Table 2 below.

**(Table 2)**

| Formula (A-2) | m21 | X21 | R16-R27 | Z21, Z22 | Z23 | n21 | n22 | n23 |
|---|---|---|---|---|---|---|---|---|
| A-2-1 | 1 | ortho-phenylene | methyl | propylene | ethylene | 1 | 1 | 40 |
| A-2-2 | 1 | meta-phenylene | methyl | propylene | ethylene | 1 | 1 | 40 |
| A-2-3 | 1 | para-phenylene | methyl | propylene | ethylene | 1 | 1 | 40 |
| A-2-4 | 1 | | methyl | propylene | ethylene | 1 | 1 | 40 |
| A-2-5 | 1 | | methyl | propylene | ethylene | 1 | 1 | 40 |
| A-2-6 | 1 | ortho-phenylene | methyl | propylene | ethylene | 1 | 1 | 100 |
| A-2-7 | 1 | meta-phenylene | methyl | propylene | ethylene | 1 | 1 | 150 |
| A-2-8 | 1 | para-phenylene | methyl | propylene | ethylene | 1 | 1 | 200 |
| A-2-9 | 1 | | ethyl | propylene | ethylene | 1 | 1 | 80 |
| A-2-10 | 1 | | methyl | propylene | ethylene | 1 | 1 | 80 |
| A-2-11 | 1 | ortho-phenylene | butyl | methylene | methylene | 5 | 5 | 40 |
| A-2-12 | 1 | meta-phenylene | phenyl | ethylene | methylene | 5 | 5 | 60 |
| A-2-13 | 1 | para-phenylene | methyl | butylene | butylene | 10 | 10 | 100 |
| A-2-14 | 1 | para-phenylene | propyl | butylene | ethylene | 10 | 10 | 20 |
| A-2-15 | 0 | - | methyl | propylene | ethylene | 1 | 1 | 40 |
| A-2-16 | 0 | - | ethyl | propylene | methylene | 1 | 1 | 40 |
| A-2-17 | 0 | - | methyl | propylene | ethylene | 1 | 1 | 40 |
| A-2-18 | 0 | - | butyl | methylene | methylene | 1 | 1 | 80 |
| A-2-19 | 0 | - | phenyl | ethylene | propylene | 5 | 5 | 60 |
| A-2-20 | 0 | - | methyl | butylene | propylene | 5 | 5 | 60 |
| A-2-21 | 0 | - | propyl | butylene | butylene | 10 | 10 | 120 |

Among those shown in Table 2, the structural units represented by the formulas (A-1-2), (A-1-3), (A-1-5), (A-1-10), (A-1-15), (A-1-17), (A-2-5), (A-2-10), (A-2-15), (A-2-16) and (A-2-17) can be suitably used.

Furthermore, each of the resin A1 and the resin A2 may have, as a terminal structure, a siloxane structure represented by the following formula (A-E):

In the formula (A-E), n⁵¹ represents the repetition number of a structure within brackets, and an average of n⁵¹ in the resin A1 or the resin A2 ranges from 20 to 60.

In the formula (B), X³¹ may be a single group or two or more groups.

Examples of the structural unit represented by the formula (B) are shown in Table 3 below.

**(Table 3)**

| Formula (B) | m31 | X31 | R31,R32 | R33,R34 | R35, R36 | R37,R38 | Y31 |
|---|---|---|---|---|---|---|---|
| B-1 | 1 | ortho-phenylene | methyl | H | H | H | propylidene |
| B-2 | 1 | meta-phenylene | methyl | H | H | H | propylidene |
| B-3 | 1 | para-phenylene | methyl | H | H | H | propylidene |
| B-4 | 1 | | methyl | H | H | H | propylidene |
| B-5 | 1 | | methyl | H | H | H | propylidene |
| B-6 | 1 | para-phenylene | methyl | H | H | H | ethylidene |
| B-7 | 1 | para-phenylene | methyl | methyl | H | H | methylene |
| B-8 | 1 | para-phenylene | H | H | H | H | phenylmethylene |
| B-9 | 1 | | H | H | H | H | single bond |
| B-10 | 1 | | methyl | H | H | H | ethylidene |
| B-11 | 1 | ortho-phenylene | methyl | methyl | H | H | single bond |
| B-12 | 1 | meta-phenylene | H | H | H | H | oxygen |
| B-13 | 1 | para-phenylene | H | H | H | H | phenylethylidene |
| B-14 | 1 | para-phenylene | H | H | H | H | propylidene |
| B-15 | 1 | para-phenylene | H | H | H | H | cyclohexylidene |
| B-16 | 0 | - | methyl | H | H | H | propylidene |
| B-17 | 0 | - | methyl | H | H | H | ethylidene |
| B-18 | 0 | - | methyl | methyl | H | H | methylene |
| B-19 | 0 | - | H | H | H | H | phenylmethylene |
| B-20 | 0 | - | H | H | H | H | single bond |
| B-21 | 0 | - | methyl | H | H | H | single bond |
| B-22 | 0 | - | methyl | methyl | H | H | single bond |
| B-23 | 0 | - | H | H | H | H | oxygen |
| B-24 | 0 | - | H | H | H | H | phenylethylidene |
| B-25 | 0 | - | H | H | H | H | propylidene |
| B-26 | 0 | - | H | H | H | H | cyclohexylidene |

In Table 3, "propylidene" indicates a 2,2-propylidene group and "phenylethylidene" indicates a 1-phenyl-1,1-ethylidene group.

Furthermore, the content of the structural unit represented by the formula (A-1) and the structural unit represented by the formula (A-2) is from 10% by mass to 40% by mass based on the total mass of the resin A1 and the resin A2. Specifically, if the resin A1 is contained but the resin A2 is not contained, {the mass of the structural unit represented by the formula (A-1)} / (the mass of the resin A1) is from 10% by mass to 40% by mass. Alternatively, if the resin A2 is contained but the resin A1 is not contained, {the mass of the structural unit represented by the formula (A-2)} / (the mass of the resin A2) is from 10% by mass to 40% by mass. If both the resin A1 and the resin A2 are contained, {the mass of the structural unit represented by the formula (A-1) + the mass of the structural unit represented by the formula (A-2)} / (the mass of the resin A1 + the mass of the resin A2) is from 10% by mass to 40% by mass. Furthermore, the content of the structural unit represented by the formula (B) is from 60% by mass to 90% by mass based on the total mass of the resin A1 and the resin A2. Specifically, if the resin A1 is contained but the resin A2 is not contained, {the mass of the structural unit represented by the formula (B)} / (the mass of the resin A1) is from 60% by mass to 90% by mass. Alternatively, if the resin A2 is contained but the resin A1 is not contained, {the mass of the structural unit represented by the formula (B)} / (the mass of the resin A2) is from 60% by mass to 90% by mass. If both the resin A1 and the resin A2 are contained, {the mass of the structural unit represented by the formula (B)} / (the mass of the resin A1 + the mass of the resin A2) is from 60% by mass to 90% by mass.

If the content of the structural unit represented by the formula (A-1) and the structural unit represented by the formula (A-2) is from 10% by mass to 40% by mass, the domains can be efficiently formed in the matrix containing the charge-transporting substance and the resin C. Therefore, the effect of relaxing the contact stress can be persistently exhibited. Furthermore, localization of the resin A1 and the resin A2 on the interface between the charge-transporting layer and the charge-generating layer can be suppressed, so as to suppress the potential variation.

Moreover, from the viewpoint of efficiently forming the domains in the matrix, the total content of the resin A1 and the resin A2 is preferably from 5% by mass to 50% by mass based on the total mass of all resins contained in the charge-transporting layer. The total content is more preferably from 10% by mass to 40% by mass.

Furthermore, as long as the effects of the present invention are not retarded, the resin A1 and the resin A2 may contain a bisphenol-derived structural unit as a structural unit apart from the structural unit represented by the formula (A-1), the structural unit represented by the formula (A-2) and the structural unit represented by the formula (B). In this case, the content of the bisphenol-derived structural unit can be 30% by mass or less based on the total mass of the resin A1 and the resin A2.

The resin A1 is a copolymer having the structural unit represented by the formula (A-1) and the structural unit represented by the formula (B). The resin A2 is a copolymer having the structural unit represented by the formula (A-2) and the structural unit represented by the formula (B). The form of copolymerization of these resins may be any one of block copolymerization, random copolymerization, alternating copolymerization.

The weight average molecular weight of the resin A1 and the resin A2 is preferably from 30,000 to 200,000 from the viewpoint of forming the domains in the matrix containing the charge-transporting substance and the resin C. The weight average molecular weight is more preferably from 40,000 to 150,000.

In the present invention, the weight average molecular weight of a resin means a weight average molecular weight in terms of polystyrene measured by a usual method, specifically, a method described in Japanese Patent Application Laid-Open No. 2007-79555.

The copolymerization ratio of the resin A1 and the copolymerization ratio of the resin A2 can be verified, as generally carried out, by a conversion method using a peak area ratio of a hydrogen atom (a hydrogen atom contained in the resins) obtained by measuring the ¹H-NMR of the resins.

The resin A1 and the resin A2 used in the present invention can be synthesized by a method described in International Publication No. WO2010/008095.

### (Resin C)

The resin C having the structural unit represented by the formula (C) will now be described. In the formula (C), X⁴¹ may be a single group or two or more groups. Y⁴¹ represents any of the groups mentioned above and can be a propylidene group.

Examples of the structural unit represented by the formula (C) are shown in Table 4 below.

**(Table 4)**

| Formula (C) | m41 | X41 | R41,R42 | R43,R44 | R45,R46 | R47,R48 | Y41 |
|---|---|---|---|---|---|---|---|
| C-1 | 1 | ortho-phenylene | methyl | H | H | H | propylidene |
| C-2 | 1 | meta-phenylene | methyl | H | H | H | propylidene |
| C-3 | 1 | para-phenylene | methyl | H | H | H | propylidene |
| C-4 | 1 | | methyl | H | H | H | propylidene |
| C-5 | 1 | | methyl | H | H | H | propylidene |
| C-6 | 1 | para-phenylene | methyl | H | H | H | ethylidene |
| C-7 | 1 | para-phenylene | methyl | methyl | H | H | methylene |
| C-8 | 1 | para-phenylene | H | H | H | H | phenylmethylene |
| C-9 | 1 | | H | H | H | H | single bond |
| C-10 | 1 | | methyl | H | H | H | ethylidene |
| C-11 | 1 | ortho-phenylene | methyl | methyl | H | H | single bond |
| C-12 | 1 | metal-phenylene | H | H | H | H | oxygen |
| C-13 | 1 | para-phenylene | H | H | H | H | phenylethylidene |
| C-14 | 1 | para-phenylene | H | H | H | H | propylidene |
| C-15 | 1 | para-phenylene | H | H | H | H | cyclohexylidene |
| C-16 | 0 | - | methyl | H | H | H | propylidene |
| C-17 | 0 | - | methyl | H | H | H | ethylidene |
| C-18 | 0 | - | methyl | methyl | H | H | methylene |
| C-19 | 0 | - | H | H | H | H | phenylmethylene |
| C-20 | 0 | - | H | H | H | H | single bond |
| C-21 | 0 | - | methyl | H | H | H | single bond |
| C-22 | 0 | - | methyl | methyl | H | H | single bond |
| C-23 | 0 | - | H | H | H | H | oxygen |
| C-24 | 0 | - | H | H | H | H | phenylethylidene |
| C-25 | 0 | - | H | H | H | H | propylidene |
| C-26 | 0 | - | H | H | H | H | cyclohexylidene |

In Table 4, "propylidene" means a 2,2-propylidene group and "phenylethylidene" means a 1-phenyl-1,1-ethylidene group.

Among those shown in Table 4, the structural units represented by any one of the formulas (C-2), (C-3), (C-4), (C-5), (C-10), (C-16), (C-18), (C-19), (C-24), (C-25) and (C-26) can be suitably used.

### (Compound D)

Next, the compound D having the structural unit represented by the formula (O-1) and the structural unit represented by the formula (0-2) will be described.

In the formula (O-1), R⁶² represents a phenyl group, a cyano group, a carbamoyl group or a group represented by the formula -COOR⁶⁴. R⁶⁴ represents a hydrogen atom, a methyl group, an ethyl group, a propyl group, an isopropyl group, a butyl group, an isobutyl group, a 2-ethylhexyl group, a nonyl group, an isononyl group, a cyclohexyl group, a 2-methoxyethyl group or a 2-hydroxyethyl group. R⁶² can be a phenyl group or a group represented by the formula -COOR⁶⁴, where R⁶⁴ can be a hydrogen atom, a methyl group, a 2-ethylhexyl group, a 2-methoxyethyl group or a 2-hydroxyethyl group.

One structural unit represented by the formula (O-1) may be singly used, or two or more of different structural units represented by the formula (O-1) shown in Table 5 below may be used together.

In the formula (0-2), R⁶³ represents a hydrogen atom or a methyl group, and n⁶¹ represents the repetition number of a structure within brackets, an average of n⁶¹ ranges from 1 to 500. One structural unit represented by the formula (0-2) may be singly used, or two or more of different structural units represented by the formula (0-2) shown in Table 6 below may be used together.

Examples of the compound D having the structural unit represented by the formula (O-1) and the structural unit represented by the formula (0-2) are shown in Tables 5 and 6 below.

**(Table 5)**

| | R⁶¹ | R⁶² | R⁶⁴ |
|---|---|---|---|
| O-1-1 | H | phenyl | - |
| O-1-2 | methyl | phenyl | - |
| O-1-3 | H | COOR⁶⁴ | methyl |
| O-1-4 | H | COOR⁶⁴ | 2-ethylhexyl |
| O-1-5 | H | COOR⁶⁴ | cyclohexyl |
| O-1-6 | H | COOR⁶⁴ | isononyl |
| O-1-7 | H | COOR⁶⁴ | 2-methoxyethyl |
| O-1-8 | methyl | COOR⁶⁴ | H |
| O-1-9 | methyl | COOR⁶⁴ | methyl |
| O-1-10 | methyl | COOR⁶⁴ | ethyl |
| O-1-11 | methyl | COOR⁶⁴ | isopropyl |
| O-1-12 | methyl | COOR⁶⁴ | cyclohexyl |
| O-1-13 | methyl | COOR⁶⁴ | 2-ethylhexyl |
| O-1-14 | methyl | COOR⁶⁴ | butyl |
| O-1-15 | methyl | COOR⁶⁴ | isobutyl |
| O-1-16 | methyl | COOR⁶⁴ | 2-methoxyethyl |
| O-1-17 | methyl | COOR⁶⁴ | 2-hydroxyethyl |
| O-1-18 | methyl | carbamoyl | - |
| O-1-19 | methyl | cyano | - |
| O-1-20 | H | carbamoyl | - |
| O-1-21 | H | cyano | - |

**(Table 6)**

| | R⁶³ | n⁶¹ |
|---|---|---|
| O-2-1 | H | 5 |
| O-2-2 | H | 10 |
| O-2-3 | H | 20 |
| O-2-4 | H | 40 |
| O-2-5 | H | 60 |
| O-2-6 | H | 80 |
| O-2-7 | H | 100 |
| O-2-8 | H | 160 |
| O-2-9 | H | 200 |
| O-2-10 | H | 300 |
| O-2-11 | H | 500 |
| O-2-12 | methyl | 5 |
| O-2-13 | methyl | 10 |
| O-2-14 | methyl | 20 |
| O-2-15 | methyl | 40 |
| O-2-16 | methyl | 60 |
| O-2-17 | methyl | 80 |
| O-2-18 | methyl | 100 |
| O-2-19 | methyl | 160 |
| O-2-20 | methyl | 200 |
| O-2-21 | methyl | 300 |
| O-2-22 | methyl | 500 |

The compound D having these structural units is commercially available from Toagosei Co., Ltd. as a silicone graft polymer. Specific examples of the commercial product include GS-30, GS-101, GS-3000, US-120, US-270, US-350, US-352, US-380 and GS-1015.

Furthermore, the compound D having these structural units can be synthesized by methods described in Japanese Patent Application Laid-Open Nos. H11-140143 and 2009-197042. From the viewpoint that the compound D can be efficiently contained in the domain containing the resin A1, the resin A2, the weight average molecular weight of the compound D is preferably from 1,000 to 150,000. The more preferably from 3,000 to 100,000. In the present invention, the compounds D were synthesized by a similar method using raw materials corresponding to Tables 5 and 6. The compositions and the weight average molecular weights of the synthesized compounds D are shown in Table 7.

**Table 7**

| Synthesis example | Compound D | Formula (O-1) | Formula (O-2) | Content (mass%) of Formula (O-1) | Content (mass%) of Formula (O-2) | Mw |
|---|---|---|---|---|---|---|
| 1 | D-1 | O-1-1 | 0-2-12 | 90 | 10 | 5000 |
| 2 | D-2 | O-1-1 | 0-2-12 | 90 | 10 | 10000 |
| 3 | D-3 | O-1-1 | 0-2-12 | 90 | 10 | 15000 |
| 4 | D-4 | O-1-1 | 0-2-12 | 90 | 10 | 30000 |
| 5 | D-5 | O-1-1 | 0-2-12 | 90 | 10 | 42000 |
| 6 | D-6 | O-1-1 | 0-2-12 | 60 | 40 | 11000 |
| 7 | D-7 | O-1-1 | 0-2-12 | 95 | 5 | 7200 |
| 8 | D-8 | O-1-1 | 0-2-13 | 80 | 20 | 12000 |
| 9 | D-9 | O-1-1 | 0-2-14 | 70 | 30 | 24000 |
| 10 | D-10 | O-1-1 | 0-2-15 | 90 | 10 | 31000 |
| 11 | D-11 | O-1-9 | 0-2-12 | 70 | 30 | 30000 |
| 12 | D-12 | O-1-9 | 0-2-12 | 70 | 30 | 45000 |
| 13 | D-13 | O-1-9 | 0-2-12 | 90 | 10 | 21000 |
| 14 | D-14 | O-1-9 | 0-2-13 | 80 | 20 | 13000 |
| 15 | D-15 | O-1-9 | 0-2-14 | 70 | 30 | 43000 |
| 16 | D-16 | O-1-9 | 0-2-15 | 60 | 40 | 26000 |
| 17 | D-17 | O-1-2 | 0-2-15 | 60 | 40 | 15000 |
| 18 | D-18 | O-1-7 | 0-2-15 | 80 | 20 | 24000 |
| 19 | D-19 | O-1-8 | 0-2-15 | 80 | 20 | 36000 |
| 20 | D-20 | O1-13 | 0-2-18 | 70 | 30 | 55000 |
| 21 | D-21 | O-1-13 | 0-2-19 | 70 | 30 | 76000 |
| 22 | D-22 | O-1-14 | 0-2-20 | 80 | 20 | 74000 |
| 23 | D-23 | O-1-15 | 0-2-21 | 70 | 30 | 80000 |
| 24 | D-24 | O-1-16 | 0-2-2 | 90 | 10 | 17000 |
| 25 | D-25 | O-1-17 | 0-2-5 | 70 | 30 | 36000 |
| 26 | D-26 | O-1-18 | 0-2-15 | 60 | 40 | 8000 |
| 27 | D-27 | O-1-19 | 0-2-15 | 80 | 20 | 15000 |
| 28 | D-28 | O-1-20 | 0-2-15 | 90 | 10 | 42000 |
| 29 | D-29 | O-1-21 | 0-2-15 | 90 | 10 | 60000 |
| 30 | D-30 | O-1-1/O-1-13=1/1 | 0-2-14 | 80 | 20 | 7500 |
| 31 | D-31 | O-1-1/O-1-13=3/1 | 0-2-16 | 80 | 20 | 27000 |
| 32 | D-32 | O-1-1/O-1-17=1/1 | 0-2-14 | 70 | 30 | 6000 |
| 33 | D-33 | O-1-1/O-1-17=3/1 | 0-2-14 | 90 | 10 | 54000 |
| 34 | D-34 | O-1-1/O-1-8/O-1-17=5/1/1 | 0-2-14 | 70 | 30 | 36000 |

In Table 7, "Formula (O-1)" means a structural unit represented by the formula (O-1) contained in each compound D. When different structural units represented by the formula (O-1) are mixedly used, the types of the structural units and a mixing ratio (in a mole ratio) are shown. "Formula (O-2)" means a structural unit represented by the formula (0-2) contained in each compound D. "Content (mass%) of formula (O-1)" means a content (% by mass) of the structural unit represented by the formula (0-1) contained in each compound D. "Content (mass%) of formula (O-2)" means a content (% by mass) of the structural unit represented by the formula (0-2) contained in each compound D. "Mw" means the weight average molecular weight of each compound D.

The content of the compound D is preferably from 1% by mass to 50% by mass based on the total mass of the resin A1 and the resin A2 because the compound D can be thus efficiently contained in the domain containing the resin A1 and the resin A2. The content is more preferably from 10% by mass to 40% by mass.

Furthermore, from the viewpoint of suppressing the potential variation in repeated use, the content of the compound D can be from 0.1% by mass to 20% by mass based on the total mass of all resins contained in the charge-transporting layer.

The charge-transporting layer of the present invention has the matrix-domain structure including the matrix containing the charge-transporting substance and the resin C, and the domains formed in the matrix and containing the compound D and at least one of the resin A1 and the resin A2.

Now, synthesis examples of the resin A1 and the resin A2 will be described.

The resin A1 and the resin A2 can be synthesized by a synthesis method described in International Publication No. WO2010/008095. Also in the present invention, resins A1 and resins A2 as shown as synthesis examples in Table 8 were synthesized by a similar method by using raw materials corresponding to the structural unit represented by the formula (A-1), the structural unit represented by the formula (A-2) and the structural unit represented by the formula (B). The compositions and the weight average molecular weights of the synthesized resins A1 and A2 are shown in Table 8. Incidentally, the resin A1 and the resin A2 may be generically designated as the "resin A."

**(Table 8)**

| Synthesis example | Resin A | Formula (A-1) or (A-2) | Formula (B) | n⁵¹ in Formula (A-E) | Content (mass%) of Formula (A-1) or (A-2) | Content (mass%) of Formula (B) | Content (mass%) of Formula (A-E) | Mw |
|---|---|---|---|---|---|---|---|---|
| 1 | Resin A(1) | A-1-5 | B-5 | - | 20 | 80 | - | 90000 |
| 2 | Resin A(2) | A-1-5 | B-5 | - | 10 | 90 | - | 100000 |
| 3 | Resin A(3) | A-1-5 | B-5 | - | 30 | 70 | - | 120000 |
| 4 | Resin A(4) | A-1-5 | B-5 | - | 40 | 60 | - | 110000 |
| 5 | Resin A(5) | A-1-5 | B-5 | - | 15 | 85 | - | 130000 |
| 6 | Resin A(6) | A-1-5 | B-5 | - | 25 | 75 | - | 80000 |
| 7 | Resin A(7) | A-1-2/A-1-3=5/5 | B-2/B-3=5/5 | - | 20 | 80 | - | 90000 |
| 8 | Resin A(8) | A-1-2/A-1-5=3/7 | B-2/B-5=3/7 | - | 30 | 70 | - | 100000 |
| 9 | Resin A(9) | A-1-3/A-1-5=1/9 | B-3/B-5=1/9 | - | 25 | 75 | - | 120000 |
| 10 | Resin A(10) | A-1-2/A-1-5=7/3 | B-3/B-10=7/3 | - | 15 | 85 | - | 110000 |
| 11 | Resin A(11) | A-1-2/A-1-5=6/4 | B-3/B-10=6/4 | - | 10 | 90 | - | 130000 |
| 12 | Resin A(12) | A-1-10 | B-5 | - | 20 | 80 | - | 80000 |
| 13 | Resin A(13) | A-1-10 | B-5 | - | 10 | 90 | - | 100000 |
| 14 | Resin A(14) | A-1-10 | B-5 | - | 30 | 70 | - | 120000 |
| 15 | Resin A(15) | A-1-10 | B-5 | - | 40 | 60 | - | 110000 |
| 16 | Resin A(16) | A-1-15 | B-23/B-26=2/8 | - | 20 | 80 | - | 90000 |
| 17 | Resin A(17) | A-1-15 | B-23/B-26=2/8 | - | 25 | 75 | - | 100000 |
| 18 | Resin A(18) | A-1-15 | B-23/B-26=2/8 | - | 30 | 70 | - | 80000 |
| 19 | Resin A(19) | A-1-15 | B-23/B-26=1/9 | - | 40 | 60 | - | 70000 |
| 20 | Resin A(20) | A-1-15 | B-23/B-26=2/8 | 40 | 10 | 80 | 10 | 100000 |
| 21 | Resin A(21) | A-1-15 | B-23/B-26=2/8 | 40 | 20 | 70 | 10 | 60000 |
| 22 | Resin A(22) | A-1-15 | B-23/B-26=2/8 | 40 | 10 | 70 | 20 | 50000 |
| 23 | Resin A(23) | A-1-15 | B-23/B-26=2/8 | 40 | 30 | 60 | 10 | 40000 |
| 24 | Resin A(24) | A-1-17 | B-23/B-26=2/8 | 40 | 10 | 60 | 30 | 30000 |
| 25 | Resin A(25) | A-2-5 | B-16 | - | 10 | 90 | - | 80000 |
| 26 | Resin A(26) | A-2-15 | B-26 | - | 20 | 80 | - | 100000 |
| 27 | Resin A(27) | A-2-15 | B-16/B-26=7/3 | - | 20 | 80 | - | 90000 |
| 28 | Resin A(28) | A-2-20 | B-16/B-24=7/3 | - | 30 | 70 | - | 70000 |
| 29 | Resin A(29) | A-2-15 | B-16 | 40 | 10 | 80 | 10 | 60000 |
| 30 | Resin A(30) | A-2-16 | B-17 | 60 | 10 | 80 | 10 | 50000 |
| 31 | Resin A(31) | A-2-17 | B-18 | 20 | 10 | 80 | 10 | 70000 |

In table 8, "Formula (A-1) or (A-2)" means a structural unit represented by the formula (A-1) contained in each resin A1 or a structural unit represented by the formula (A-2) contained in each resin A2. If a plurality of structural units represented by the formula (A-1) or a plurality of structural units represented by the formula (A-2) are mixedly used, the types of the structural units and a mixing ratio (in a mole ratio) are shown. "Formula (B)" means a structural unit represented by the formula (B) contained in each resin A1 or A2. If a plurality of structural units represented by the formula (B) are mixedly used, the types of the structural units and a mixing ratio (in a mole ratio) are shown. Besides, "n⁵¹ in Formula (A-E)" means an average of the repetition number in a structural unit represented by the formula (A-E) contained in each resin A1 or A2. "Content (mass%) of Formula (A-1) or (A-2)" means the content (% by mass) of a structural unit represented by the formula (A-1) in each resin A1 or the content (% by mass) of a structural unit represented by the formula (A-2) in each resin A2. "Content (mass%) of Formula (B)" means the content (% by mass) of a structural unit represented by the formula (B) in each resin A1 or A2. "Content (mass%) of Formula (A-E)" means the content (% by mass) of a structural unit represented by the formula (A-E) in each resin A1 or A2. "Mw" means the weight average molecular weight of each resin A1 or A2.

The charge-transporting layer corresponding to the surface layer of the electrophotographic photosensitive member contains at least one of the resin A1 and the resin A2, and the resin C, and another resin may be mixedly used. Examples of another resin that may be mixedly used include an acrylic resin, a polyester resin and a polycarbonate resin.

Furthermore, from the viewpoint of efficiently forming the matrix-domain structure, it is preferable that the resin C contains neither a structural unit represented by the formula (A-1) nor a structural unit represented by the formula (A-2).

The charge-transporting layer contains the charge-transporting substance. Examples of the charge-transporting substance include a triarylamine compound, a hydrazone compound, butadiene compound and an enamine compound. One of these charge-transporting substances may be singly used, or two or more of these may be used together. Among these compounds, a triarylamine compound can be suitably used as the charge-transporting substance from the viewpoint of improvement of electrophotographic characteristics.

Specific examples of the charge-transporting substance are as follows:

The ratio between the charge-transporting substance and the resins is preferably 4:10 to 20:10 (in a mass ratio) and more preferably 5:10 to 12:10 (in a mass ratio). Furthermore, the content of the charge-transporting substance can be from 25% by mass to 70% by mass based on the total mass of the charge-transporting layer.

Examples of a solvent to be used in the charge-transporting layer coating solution include a ketone solvent, an ester solvent, an ether solvent and an aromatic hydrocarbon solvent. One of these solvents may be singly used, or a mixture of two or more of these may be used. Among these solvents, an ether solvent or an aromatic hydrocarbon solvent can be suitably used from the viewpoint of resin solubility.

The thickness of the charge-transporting layer is preferably from 5 µm to 50 µm, and more preferably from 10 µm to 35 µm.

Besides, an antioxidant, a UV absorber, a plasticizer may be added to the charge-transporting layer as occasion demands.

The charge-transporting layer can be formed from a coating film of the charge-transporting layer coating solution, which is prepared by dissolving, in the solvent, at least one selected from the group consisting of the resin A1 and the resin A2, the compound D, the charge-transporting substance and the resin C.

Next, the structure of the electrophotographic photosensitive member of the present invention will be described.

The electrophotographic photosensitive member includes a support, a charge-generating layer formed on the support and a charge-transporting layer formed on the charge-generating layer. Furthermore, the charge-transporting layer is a surface layer (an uppermost layer) of the electrophotographic photosensitive member. Moreover, the charge-transporting layer may have a layered structure, and in that case, at least a surfacemost(outermost) portion of the charge-transporting layer has the matrix-domain structure.

FIGS. 2A and 2B are diagrams illustrating examples of a layered structure of the electrophotographic photosensitive member of the present invention. In FIGS. 2A and 2B, a reference numeral 101 denotes a support, a reference numeral 102 denotes a charge-generating layer, a reference numeral 103 denotes a charge-transporting layer (or a first charge-transporting layer) and a reference numeral 104 denotes a second charge-transporting layer.

As for the shape of the electrophotographic photosensitive member, a cylindrical electrophotographic photosensitive member obtained by forming a photosensitive layer (a charge-generating layer and a charge-transporting layer) on a cylindrical support is generally widely used, but the electrophotographic photosensitive member can be in the shape of a belt, a sheet.

### (Support)

The support can be one having conductivity (namely, a conductive support), and a support made of a metal such as aluminum, an aluminum alloy or stainless steel can be used. As a support made of aluminum or an aluminum alloy, an ED tube, an EI tube, or a support obtained by subjecting such a tube to cutting, electrolytic composite polishing, or wet or dry honing can be used. Alternatively, a metal support or a resin support on which a film of aluminum, an aluminum alloy or an indium oxide-tin oxide alloy is formed by vacuum deposition can be used. The surface of the support may be subjected to cutting, surface roughening, an alumite treatment.

Further alternatively, a support obtained by impregnating a resin with conductive particles such as carbon black, tin oxide particles, titanium oxide particles or silver particles, or a plastic support containing a conductive resin can be used.

A conductive layer may be provided between the support and an undercoat layer described later or the charge-generating layer for purposes of suppressing interference fringe derived from scattering of laser beams and covering a scar of the support. This conductive layer is formed by using a conductive layer coating solution obtained by dispersing conductive particles in a resin.

Examples of the conductive particles include carbon black, acetylene black, a metal powder of aluminum, nickel, iron, nichrome, copper, zinc, silver and a metal oxide powder of conductive tin oxide or ITO.

Examples of the resin used for the conductive layer include a polyester resin, a polycarbonate resin, a polyvinyl butyral resin, an acrylic resin, a silicone resin, an epoxy resin, a melamine resin, a urethane resin, a phenol resin and an alkyd resin.

Examples of a solvent used in the conductive layer coating solution include an ether solvent, an alcohol solvent, a ketone solvent and an aromatic hydrocarbon solvent.

The thickness of the conductive layer is preferably from 0.2 µm to 40 µm, more preferably from 1 µm to 35 µm and further preferably from 5 µm to 30 µm.

Between the support or the conductive layer and the charge-generating layer, an undercoat layer may be provided.

The undercoat layer can be formed by forming a coating film by applying, on the conductive layer, an undercoat layer coating solution containing a resin, and drying or curing the coating film.

Examples of the resin used for the undercoat layer include polyacrylic acids, methyl cellulose, ethyl cellulose, a polyamide resin, a polyimide resin, a polyamideimide resin, a polyamic acid resin, a melamine resin, an epoxy resin, a polyurethane resin and a polyolefin resin. The resin for the undercoat layer can be a thermoplastic resin. Specifically, a thermoplastic polyamide resin or polyolefin resin can be suitably used. As the polyamide resin, low-crystalline or non-crystalline copolymer nylon that can be applied in a solution state can be suitably used. The polyolefin resin can be in a state usable as a particle dispersion. Besides, the polyolefin resin can be dispersed in an aqueous medium.

The thickness of the undercoat layer is preferably from 0.05 µm to 7 µm and more preferably from 0.1 µm to 2 µm.

Furthermore, the undercoat layer may contain semiconductive particles, an electron transporting substance or an electron accepting substance.

### (Charge-generating layer)

The charge-generating layer is provided on the support, the conductive layer or the undercoat layer.

Examples of a charge-generating substance used in the electrophotographic photosensitive member include an azo pigment, a phthalocyanine pigment, an indigo pigment and a perylene pigment. One of these charge-generating substances may be singly used, or two or more of these may be used together. Among these substances, metal phthalocyanines such as oxytitanium phthalocyanine, hydroxygallium phthalocyanine and chlorogallium phthalocyanine can be particularly suitably used because of their high sensitivity.

Examples of a resin used for the charge-generating layer include a polycarbonate resin, a polyester resin, a butyral resin, a polyvinyl acetal resin, an acrylic resin, a vinyl acetate resin and a urea resin. Among these resins, a butyral resin can be particularly suitably used. One of these resins may be singly used, or one, two or more of these may be used in the form of a mixture or a copolymer.

The charge-generating layer can be formed by forming a coating film of a charge-generating layer coating solution obtained by dispersing a charge-generating substance with a resin and a solvent, and drying the thus obtained coating film. Alternatively, the charge-generating layer may be formed as a deposited film of a charge-generating substance.

As a dispersing method, a method using, for example, a homogenizer, ultrasonic waves, a ball mill, a sand mill, an attritor or a roll mill can be employed.

The ratio between the charge-generating substance and the resin is preferably 1:10 to 10:1 (in a mass ratio) and particularly more preferably 1:1 to 3:1 (in a mass ratio).

Examples of the solvent used in the charge-generating layer coating solution include an alcohol solvent, a sulfoxide solvent, a ketone solvent, an ether solvent, an ester solvent and an aromatic hydrocarbon solvent.

The thickness of the charge-generating layer is preferably 5 µm or less and more preferably from 0.1 µm to 2 µm.

Furthermore, various agents such as a sensitizing agent, an antioxidant, a UV absorber and a plasticizer may be added to the charge-generating layer as occasion demands. Moreover, the charge-generating layer may contain an electron transporting substance or an electron accepting substance, so as not to stagnate the flow of charge in the charge-generating layer.

The charge-transporting layer is provided on the charge-generating layer.

Various additives may be added to each layer of the electrophotographic photosensitive member. Examples of the additives include an antidegradant such as an antioxidant, a UV absorber or a light stabilizer, and fine particles such as organic fine particles or inorganic fine particles. Examples of the antidegradant include a hindered phenol antioxidant, a hindered amine light stabilizer, a sulfur atom-containing antioxidant and a phosphorus atom-containing antioxidant. Examples of the organic fine particles include polymer resin particles such as fluorine atom-containing resin particles, polystyrene fine particles and polyethylene resin particles. Examples of the inorganic fine particles include fine particles of metal oxides such as silica and alumina.

In applying the coating solution for each layer, an application method such as a dip applying method (a dip-coating method), a spray coating method, a spinner coating method, a roller coating method, a Meyer bar coating method or a blade coating method can be employed.

Furthermore, the surface of the charge-transporting layer, that is, the surface layer of the electrophotographic photosensitive member, may be provided with irregularities (recesses and protrusions). The irregularities can be formed by any of known methods. Examples of the method for forming the irregularities include the following: A method in which recesses are formed by blasting abrasive particles against the surface; a method in which irregularities are formed by bringing a mold having an irregular surface into contact with the surface with a pressure; a method in which recesses are formed by forming dew on a surface of the coating film of an applied surface layer coating solution and then drying the dew; and a method in which recesses are formed by irradiating the surface with laser beams. Among these methods, the method in which irregularities are formed by bringing a mold having an irregular surface into contact with the surface of the electrophotographic photosensitive member with a pressure can be suitably employed. Alternatively, the method in which recesses are formed by forming dew on a surface of the coating film of an applied surface layer coating solution and then drying the dew can be suitably employed.

### (Electrophotographic apparatus)

FIG. 1 illustrates an example of the schematic structure of an electrophotographic apparatus provided with a process cartridge including an electrophotographic photosensitive member.

In FIG. 1, a reference numeral 1 denotes a cylindrical electrophotographic photosensitive member, which is driven to rotate around an axis 2 in a direction illustrated with an arrow at a prescribed circumferential speed. The surface of the electrophotographic photosensitive member 1 thus driven to rotate is uniformly charged to a positive or negative prescribed potential by charging device 3 (primary charging device, such as a charging roller). Subsequently, the electrophotographic photosensitive member 1 is irradiated with exposing light 4 (image exposing light) output from exposing device (not shown) for slit exposure, laser beam scanning. In this manner, an electrostatically latent image corresponding to a desired image is successively formed on the surface of the electrophotographic photosensitive member 1.

The electrostatically latent image formed on the surface of the electrophotographic photosensitive member 1 is developed into a toner image by a toner contained in a developer supplied by developing device 5. Subsequently, the toner image formed and carried on the surface of the electrophotographic photosensitive member 1 is successively transferred onto a transfer material P (such as paper) by a transfer bias applied by transferring device 6 (such as a transfer roller). Incidentally, the transfer material P is taken out of transfer material supplying device (not shown) in synchronization with the rotation of the electrophotographic photosensitive member 1 to be fed to a portion (a contact portion) between the electrophotographic photosensitive member 1 and the transferring device 6.

The transfer material P onto which the toner image has been transferred is separated from the surface of the electrophotographic photosensitive member 1 to be introduced into fixing device 8, in which the image is fixed, and thus, the resultant is output as an image formed product (a printed or copied product) to the outside of the apparatus.

After transferring the toner image, the surface of the electrophotographic photosensitive member 1 is cleaned by cleaning device 7 (such as a cleaning blade) so as to remove remaining developer (toner). Subsequently, the electrophotographic photosensitive member is subjected to a discharging treatment with pre-exposing light (not shown) emitted by pre-exposing device (not shown), so as to be repeatedly used for image formation. Incidentally, if the charging device 3 is contact charging device using a charging roller as illustrated in FIG. 1, pre-exposure is not always necessary.

Among the components such as the electrophotographic photosensitive member 1, the charging device 3, the developing device 5, the transferring device 6 and the cleaning device 7, some are housed in a vessel to be integrated as a process cartridge. This process cartridge may be constructed to be removably provided in a main body of an electrophotographic apparatus such as a copying machine or a laser beam printer. In FIG. 1, the electrophotographic photosensitive member 1, the charging device 3, the developing device 5 and the cleaning device 7 are integrally supported as a cartridge, so as to provide a process cartridge 9 that may be removably provided in a main body of an electrophotographic apparatus by using guiding device 10 such as a rail provided on the main body of the electrophotographic apparatus.

### Examples

The present invention will now be described in more detail with reference to specific examples. In the following examples, the term "part(s)" means "part(s) by mass."

### (Example 1)

An aluminum cylinder having a diameter of 24 mm and a length of 257 mm was used as a support (a conductive support).

Next, a conductive layer coating solution was prepared by using 10 parts of SnO₂-coated barium sulfate particles (used as conductive particles), 2 parts of titanium oxide particles (used as a pigment for adjusting resistance), 6 parts of a phenol resin, 0.001 part of silicone oil (used as a leveling agent) and a mixed solvent of 4 parts of methanol and 16 parts of methoxypropanol. The conductive layer coating solution was dip-coated on the support to obtain a coating film, and the coating film was cured (thermally cured) at 140°C for 30 minutes, thereby forming a conductive layer with a thickness of 15 µm.

Next, an undercoat layer coating solution was prepared by dissolving 3 parts of N-methoxymethylated nylon and 3 parts of copolymer nylon in a mixed solvent of 65 parts of methanol and 30 parts of n-butanol. The undercoat layer coating solution was dip-coated on the conductive layer to form a coating film, and the coating film was dried at 100°C for 10 minutes, thereby forming an undercoat layer with a thickness of 0.7 µm.

Next, 10 parts of hydroxygallium phthalocyanine (having intensive peaks, in CuKα characteristic X-ray diffraction, at the Bragg angle 2θ ± 0.2° of 7.5°, 9.9°, 16.3°, 18.6°, 25.1° and 28.3°) was added, as a charge-generating substance, to a solution of 5 parts of a polyvinyl butyral resin (trade name: S-lec BX-1, manufactured by Sekisui Chemical Co., Ltd.) dissolved in 250 parts of cyclohexanone. The resulting solution was subjected to dispersion by using a sand mill apparatus using glass beads with a diameter of 1 mm in an atmosphere of 23 ± 3°C for 1 hour. After the dispersion, 250 parts of ethyl acetate was added to the resulting solution, thereby preparing a charge-generating layer coating solution. The charge-generating layer coating solution was dip-coated on the undercoat layer to form a coating film, and the coating film was dried at 100°C for 10 minutes, thereby forming a charge-generating layer with a thickness of 0.26 µm.

Next, a charge-transporting layer coating solution was prepared by dissolving, in a mixed solvent of 30 parts of dimethoxymethane and 50 parts of ortho-xylene, 9 parts of a compound represented by the formula (E-1) (used as a charge-transporting substance), 1 part of a compound represented by the formula (E-2) (used as a charge-transporting substance), 3 parts of the resin A(1) synthesized as Synthesis Example 1, 7 parts of a resin C (having a weight average molecular weight of 120,000) containing a structural unit represented by the formula (C-2) and a structural unit represented by the formula (C-3) in a mole ratio of 5:5, and 0.15 part of a compound D (D-4).

This charge-transporting layer coating solution was dip-coated on the charge-generating layer to form a coating film, and the coating film was dried at 120°C for 1 hour, thereby forming a charge-transporting layer with a thickness of 16 µm. The thus formed charge-transporting layer was verified to have domains that contain the resin A(1) and the compound D and are formed in a matrix containing the charge-transporting substances and the resin C.

In this manner, the electrophotographic photosensitive member having the charge-transporting layer as a surface layer was produced. The compositions of the compound D and the resins contained in the charge-transporting layer are shown in Table 9.

Next, evaluation will be described.

The evaluation was made on variation in a potential of a light portion (potential variation) caused in repeated use for making 5,000 copies, relative values of torque obtained at an initial stage and after the repeated use for making 5,000 copies, and observation of the surface of the electrophotographic photosensitive member in measuring the torque.

### <Evaluation of potential variation>

As an evaluation apparatus, a laser beam printer, Color Laser JET CP4525dn manufactured by Hewlett-Packard was used. The evaluation was performed under environment of a temperature of 23°C and relative humidity of 50%. Exposure (image exposure) of a laser source of 780 nm of the evaluation apparatus was set so that light quantity of 0.37 µJ/cm² could be attained on the surface of the electrophotographic photosensitive member. Surface potentials (a dark portion potential and a light portion potential) of the electrophotographic photosensitive member were measured in a position of a developing device with the developing device replaced with a jig fixed to have a potential measuring probe in a position away by 130 mm from the end of the electrophotographic photosensitive member. With the dark portion potential of an unexposed portion of the electrophotographic photosensitive member set to -500 V, laser beams were irradiated for measuring a light portion potential resulting from light attenuation from the dark portion potential. Furthermore, A4-size regular paper was used for continuously outputting 5,000 copies, and variation in the light portion potential caused through this continuous operation was evaluated. A test chart having a printing ratio of 5% was used. The result is shown in a column of "Potential variation" of Table 12.

### <Evaluation of torque relative value>

A driving current value (a current value A) of a rotary motor for the electrophotographic photosensitive member was measured under the same conditions as those employed for the evaluation of the potential variation. This is evaluation of the quantity of contact stress caused between the electrophotographic photosensitive member and a cleaning blade. The magnitude of the obtained current value corresponds to the magnitude of the quantity of contact stress caused between the electrophotographic photosensitive member and the cleaning blade.

Furthermore, an electrophotographic photosensitive member to be used as a control in measuring a torque relative value was produced as follows: The resin A(1) used as the resin for the charge-transporting layer of the electrophotographic photosensitive member of Example 1 was replaced with a resin C containing a structural unit represented by the formula (C-2) and a structural unit represented by the formula (C-3) in a mole ratio of 5:5. An electrophotographic photosensitive member was produced in the same manner as in Example 1 except that the compound D was not used and the resin C alone was used as the resin, and the resultant was used as a control electrophotographic photosensitive member.

The thus produced control electrophotographic photosensitive member was used for measuring a driving current value (a current value B) of a rotary motor for the electrophotographic photosensitive member in the same manner as in Example 1.

The ratio between the driving current value (the current value A) of the rotary motor for the electrophotographic photosensitive member containing the resin A1 or the resin A2 and the driving current value (the current value B) of the rotary motor for the electrophotographic photosensitive member not containing the resin A1 and the resin A2 thus measured was calculated. The calculated value of (the current value A) / (the current value B) was compared as a torque relative value. This torque relative value corresponds to the degree of reduction of the quantity of the contact stress caused between the electrophotographic photosensitive member and the cleaning blade, and as the torque relative value is smaller, the degree of the reduction of the quantity of the contact stress caused between the electrophotographic photosensitive member and the cleaning blade is larger. The result is shown in a column of "Initial torque relative value" of Table 12.

Subsequently, A4-size regular paper was used for continuously outputting 5,000 copies. A test chart with a printing ratio of 5% was used. Thereafter, a torque relative value attained after the repeated use for making 5,000 copies was measured. The torque relative value attained after the repeated use for making 5,000 copies was measured in the same manner as the initial torque relative value. In this case, the control electrophotographic photosensitive member was also used for repeatedly outputting 5,000 copies, and a driving current value of the rotary motor obtained in the repeated use was used for calculating a torque relative value attained after the repeated use for making 5,000 copies. The result is shown in a column of "Torque relative value after making 5000 copies" of Table 12.

### <Evaluation of matrix-domain structure>

In the electrophotographic photosensitive member produced as described above, a cross-section of the charge-transporting layer obtained by vertically cutting the charge-transporting layer was observed with an ultradeep profile measuring microscope VK-9500 (manufactured by Keyence Corporation). In the observation, the magnification of an objective lens was set to 50×, an area of 100 µm square (10,000 µm²) on the surface of the electrophotographic photosensitive member was observed as an observation field of view, and maximum diameters of 100 domains formed in and randomly selected in the observation field of view were measured. An average was calculated as a number average particle size based on the obtained maximum diameters. The result is shown in Table 12.

### (Examples 2 to 20)

Electrophotographic photosensitive members were produced in the same manner as in Example 1 except that a compound D was changed as shown in Table 9, and the produced electrophotographic photosensitive members were evaluated in the same manner as in Example 1. It was verified, in the charge-transporting layer of each of the electrophotographic photosensitive members, that domains containing the resin A1 and the compound D were formed in a matrix containing the charge-transporting substance and the resin C. The results are shown in Table 12.

Incidentally, the weight average molecular weight of the resin C was:
(C-2)/(C-3) = 5/5 (in a mole ratio): 120,000.

### (Examples 21 to 30)

Electrophotographic photosensitive members were produced in the same manner as in Example 1 except that a resin C used in the charge-transporting layer was changed as shown in Table 9, and the produced electrophotographic photosensitive members were evaluated in the same manner as in Example 1. It was verified, in the charge-transporting layer of each of the electrophotographic photosensitive members, that domains containing the resin A1 and the compound D were formed in a matrix containing the charge-transporting substance and the resin C. The results are shown in Table 12.

Incidentally, the weight average molecular weights of the resins C were as follows:
(C-10): 100,000;
(C-5): 110,000;
(C-2)/(C-5) = 3/7 (in a mole ratio): 110,000;
(C-2)/(C-10) = 7/3 (in a mole ratio): 120,000;
(C-16): 140,000;
(C-19): 160,000;
(C-24): 130,000;
(C-25): 140,000; and
(C-26): 130, 000.

### (Examples 31 to 48)

Electrophotographic photosensitive members were produced in the same manner as in Example 1 except that a resin A1, a resin C and a compound D were changed as shown in Table 9, and the produced electrophotographic photosensitive members were evaluated in the same manner as in Example 1. It was verified, in the charge-transporting layer of each of the electrophotographic photosensitive members, that domains containing the resin A1 and the compound D were formed in a matrix containing the charge-transporting substance and the resin C. The results are shown in Table 12.

Incidentally, the weight average molecular weights of the resins C were as follows:
(C-4): 100,000; and
(C-18): 140,000.

### (Examples 49 to 95)

Electrophotographic photosensitive members were produced in the same manner as in Example 1 except that a resin A1, a resin A2, a resin C and a compound D were changed as shown in Table 10, and the produced electrophotographic photosensitive members were evaluated in the same manner as in Example 1. It was verified, in the charge-transporting layer of each of the electrophotographic photosensitive members, that domains containing the resin A1, the resin A2 and the compound D were formed in a matrix containing the charge-transporting substance and the resin C. The results are shown in Table 13.

### (Comparative Example 1)

An electrophotographic photosensitive member was produced in the same manner as in Example 1 except that the resin A(1) and the compound D (D-2) were not used but a resin C containing a structural unit represented by the formula (C-2) and a structural unit represented by the formula (C-3) in a mole ratio of 5:5 was used instead. Since the charge-transporting layer of this electrophotographic photosensitive member contains neither a resin A1 nor a compound D, a matrix-domain structure was not found in the charge-transporting layer. The electrophotographic photosensitive member was evaluated in the same manner as in Example 1. The result is shown in Table 14.

### (Comparative Examples 2 to 18)

Electrophotographic photosensitive members were produced in the same manner as in Comparative Example 1 except that a resin C and a compound D were changed as shown in Table 11. Since the charge-transporting layer of each of these electrophotographic photosensitive members does not contain the resin A1, a matrix-domain structure was not found in the charge-transporting layer. The electrophotographic photosensitive members were evaluated in the same manner as in Example 1. The results are shown in Table 14.

### (Comparative Example 19)

An electrophotographic photosensitive member was produced in the same manner as in Example 1 except that the compound D was replaced with dimethylpolysiloxane (KF96, manufactured by Shin-Etsu Chemical Co., Ltd.). It was verified that domains were formed in a matrix. The electrophotographic photosensitive member was evaluated in the same manner as in Example 1. The result is shown in Table 14. Incidentally, dimethylpolysiloxane has a polysiloxane structure in a main chain, and in addition, substituents on a silicon atom of siloxane are all methyl groups, and hence the dimethylpolysiloxane is a compound having a different structure from the compound D of the present invention.

### (Comparative Examples 20 to 24)

Electrophotographic photosensitive members were produced in the same manner as in Comparative Example 19 except that the resin A1 and the resin C used in Comparative Example 19 were changed as shown in Table 11 and that the compound D was replaced with dimethylpolysiloxane (KF96). It was verified that domains were formed in a matrix. The electrophotographic photosensitive members were evaluated in the same manner as in Example 1. The results are shown in Table 14.

**(Table 9)**

| Example | Resin A | Resin C | Resin A/resin C mixing ratio | Compound D | Mass% of compound D to resin A |
|---|---|---|---|---|---|
| 1 | Resin A(1) | C-2/C-3=5/5 | 3/7 | D-2 | 5 |
| 2 | Resin A(1) | C-2/C-3=5/5 | 3/7 | D-2 | 20 |
| 3 | Resin A(1) | C-2/C-3=5/5 | 3/7 | D-2 | 30 |
| 4 | Resin A(1) | C-2/C-3=5/5 | 3/7 | D-2 | 40 |
| 5 | Resin A(1) | C-2/C-3=5/5 | 3/7 | D-11 | 5 |
| 6 | Resin A(1) | C-2/C-3=5/5 | 3/7 | D-11 | 40 |
| 7 | Resin A(1) | C-2/C-3=5/5 | 3/7 | D-32 | 5 |
| 8 | Resin A(1) | C-2/C-3=5/5 | 3/7 | D-32 | 40 |
| 9 | Resin A(1) | C-2/C-3=5/5 | 3/7 | D-1 | 5 |
| 10 | Resin A(1) | C-2/C-3=5/5 | 3/7 | D-1 | 40 |
| 11 | Resin A(1) | C-2/C-3=5/5 | 3/7 | D-3 | 5 |
| 12 | Resin A(1) | C-2/C-3=5/5 | 3/7 | D-3 | 40 |
| 13 | Resin A(1) | C-2/C-3=5/5 | 3/7 | D-12 | 5 |
| 14 | Resin A(1) | C-2/C-3=5/5 | 3/7 | D-12 | 40 |
| 15 | Resin A(1) | C-2/C-3=5/5 | 3/7 | D-15 | 5 |
| 16 | Resin A(1) | C-2/C-3=5/5 | 3/7 | D-15 | 40 |
| 17 | Resin A(1) | C-2/C-3=5/5 | 3/7 | D-19 | 5 |
| 18 | Resin A(1) | C-2/C-3=5/5 | 3/7 | D-19 | 40 |
| 19 | Resin A(1) | C-2/C-3=5/5 | 3/7 | D-34 | 5 |
| 20 | Resin A(1) | C-2/C-3=5/5 | 3/7 | D-34 | 40 |
| 21 | Resin A(1) | C-10 | 3/7 | D-2 | 20 |
| 22 | Resin A(1) | C-5 | 3/7 | D-2 | 30 |
| 23 | Resin A(1) | C-2/C-5=3/7 | 3/7 | D-2 | 20 |
| 24 | Resin A(1) | C-2/C-10=7/3 | 3/7 | D-2 | 30 |
| 25 | Resin A(1) | C-16 | 3/7 | D-2 | 20 |
| 26 | Resin A(1) | C-19 | 3/7 | D-2 | 30 |
| 27 | Resin A(1) | C-24 | 3/7 | D-2 | 20 |
| 28 | Resin A(1) | C-25 | 3/7 | D-2 | 30 |
| 29 | Resin A(1) | C-26 | 3/7 | D-2 | 30 |
| 30 | Resin A(2) | C-2/C-3=5/5 | 4/6 | D-2 | 30 |
| 31 | Resin A(3) | C-10 | 2/8 | D-11 | 20 |
| 32 | Resin A(4) | C-4 | 1/9 | D-1 | 20 |
| 33 | Resin A(5) | C-2/C-5=3/7 | 3/7 | D-19 | 20 |
| 34 | Resin A(6) | C-2/C-10=7/3 | 3/7 | D-34 | 20 |
| 35 | Resin A(7) | C-18 | 3/7 | D-2 | 20 |
| 36 | Resin A(8) | C-19 | 3/7 | D-11 | 20 |
| 37 | Resin A(9) | C-24 | 3/7 | D-1 | 20 |
| 38 | Resin A(10) | C-25 | 3/7 | D-19 | 20 |
| 39 | Resin A(11) | C-26 | 3/7 | D-34 | 20 |
| 40 | Resin A(12) | C-2/C-3=5/5 | 3/7 | D-2 | 30 |
| 41 | Resin A(12) | C-2/C-3=5/5 | 3/7 | D-11 | 30 |
| 42 | Resin A(12) | C-2/C-3=5/5 | 3/7 | D-1 | 30 |
| 43 | Resin A(12) | C-2/C-3=5/5 | 3/7 | D-19 | 30 |
| 44 | Resin A(12) | C-2/C-3=5/5 | 3/7 | D-34 | 30 |
| 45 | Resin A(12) | C-26 | 3/7 | D-2 | 20 |
| 46 | Resin A(13) | C-16 | 3/7 | D-1 | 20 |
| 47 | Resin A(14) | C-19 | 3/7 | D-19 | 20 |
| 48 | Resin A(15) | C-24 | 3/7 | D-34 | 20 |

**(Tables 10)**

| Example | Resin A | Resin C | Resin A/resin C mixing ratio | Compound D | Mass% of compound D to resin A |
|---|---|---|---|---|---|
| 49 | Resin A(16) | C-26 | 3/7 | D-2 | 5 |
| 50 | Resin A(16) | C-26 | 3/7 | D-2 | 20 |
| 51 | Resin A(16) | C-26 | 3/7 | D-2 | 30 |
| 52 | Resin A(16) | C-26 | 3/7 | D-2 | 40 |
| 53 | Resin A(16) | C-26 | 3/7 | D-11 | 5 |
| 54 | Resin A(16) | C-26 | 3/7 | D-11 | 40 |
| 55 | Resin A(16) | C-16 | 3/7 | D-32 | 5 |
| 56 | Resin A(16) | C-19 | 3/7 | D-32 | 40 |
| 57 | Resin A(16) | C-24 | 3/7 | D-1 | 5 |
| 58 | Resin A(16) | C-25 | 3/7 | D-1 | 40 |
| 59 | Resin A(16) | C-16 | 3/7 | D-3 | 5 |
| 60 | Resin A(16) | C-19 | 3/7 | D-3 | 40 |
| 61 | Resin A(16) | C-24 | 3/7 | D-12 | 5 |
| 62 | Resin A(16) | C-25 | 3/7 | D-12 | 40 |
| 63 | Resin A(16) | C-2/C-3=5/5 | 3/7 | D-15 | 5 |
| 64 | Resin A(16) | C-10 | 3/7 | D-15 | 40 |
| 65 | Resin A(16) | C-5 | 3/7 | D-19 | 5 |
| 66 | Resin A(16) | C-2/C-5=3/7 | 3/7 | D-19 | 40 |
| 67 | Resin A(16) | C-2/C-10=7/3 | 3/7 | D-34 | 5 |
| 68 | Resin A(16) | C-26 | 4/6 | D-34 | 40 |
| 69 | Resin A(17) | C-26 | 3/7 | D-1 | 30 |
| 70 | Resin A(18) | C-26 | 3/7 | D-15 | 20 |
| 71 | Resin A(19) | C-26 | 3/7 | D-34 | 30 |
| 72 | Resin A(20) | C-26 | 3/7 | D-2 | 30 |
| 73 | Resin A(20) | C-26 | 3/7 | D-2 | 20 |
| 74 | Resin A(20) | C-26 | 3/7 | D-2 | 30 |
| 75 | Resin A(20) | C-16 | 3/7 | D-2 | 20 |
| 76 | Resin A(20) | C-19 | 3/7 | D-2 | 30 |
| 77 | Resin A(20) | C-24 | 3/7 | D-2 | 20 |
| 78 | Resin A(20) | C-25 | 3/7 | D-2 | 30 |
| 79 | Resin A(20) | C-2/C-3=5/5 | 3/7 | D-2 | 20 |
| 80 | Resin A(20) | C-2/C-3=5/5 | 3/7 | D-2 | 30 |
| 81 | Resin A(20) | C-10 | 3/7 | D-3 | 10 |
| 82 | Resin A(20) | C-4 | 3/7 | D-3 | 40 |
| 83 | Resin A(20) | C-2/C-5=3/7 | 3/7 | D-19 | 10 |
| 84 | Resin A(20) | C-2/C-10=7/3 | 3/7 | D-19 | 40 |
| 85 | Resin A(21) | C-18 | 3/7 | D-11 | 30 |
| 86 | Resin A(22) | C-19 | 3/7 | D-1 | 20 |
| 87 | Resin A(23) | C-24 | 3/7 | D-15 | 30 |
| 88 | Resin A(24) | C-25 | 3/7 | D-34 | 20 |
| 89 | Resin A(25) | C-2/C-3=5/5 | 3/7 | D-2 | 30 |
| 90 | Resin A(26) | C-2/C-3=5/5 | 3/7 | D-11 | 20 |
| 91 | Resin A(27) | C-10 | 3/7 | D-1 | 30 |
| 92 | Resin A(28) | C-5 | 3/7 | D-15 | 20 |
| 93 | Resin A(29) | C-2/C-5=3/7 | 3/7 | D-34 | 30 |
| 94 | Resin A(30) | C-2/C-10=7/3 | 3/7 | D-2 | 20 |
| 95 | Resin A(31) | C-26 | 3/7 | D-2 | 30 |

**(Table 11)**

| Comparative Example | A Resin A | Resin C | Resin A/resin C mixing ratio | Compound D | Mass%of Mass% of compound D to resin A |
|---|---|---|---|---|---|
| 1 | - | C-2/C-3=5/5 | - | - | - |
| 2 | - | C-2/C-3=5/5 | - | D-34 | 5 |
| 3 | - | C-2/C-3=5/5 | - | D-2 | 5 |
| 4 | - | C-2/C-3=5/5 | - | D-11 | 5 |
| 5 | - | C-2/C-3=5/5 | - | D-32 | 5 |
| 6 | - | C-2/C-3=5/5 | - | D-1 | 5 |
| 7 | - | C-2/C-3=5/5 | - | D-3 | 5 |
| 8 | - | C-2/C-3=5/5 | - | D-12 | 5 |
| 9 | - | C-2/C-3=5/5 | - | D-15 | 5 |
| 10 | - | C-10 | - | D-2 | 5 |
| 11 | - | C-5 | - | D-2 | 5 |
| 12 | - | C-2/C-5=3/7 | - | D-2 | 5 |
| 13 | - | C-2/C-10=7/3 | - | D-2 | 5 |
| 14 | - | C-16 | - | D-2 | 5 |
| 15 | - | C-19 | - | D-2 | 5 |
| 16 | - | C-24 | - | D-2 | 5 |
| 17 | - | C-25 | - | D-2 | 5 |
| 18 | - | C-26 | - | D-2 | 5 |
| 19 | Resin A(1) | C-2/C-3=5/5 | 3/7 | KF96* | 10 |
| 20 | Resin A(1) | C-26 | 3/7 | KF96* | 40 |
| 21 | Resin A(12) | C-2/C-5=3/7 | 3/7 | KF96* | 10 |
| 22 | Resin A(16) | C-19 | 3/7 | KF96* | 40 |
| 23 | Resin A(16) | C-5 | 3/7 | KF96* | 10 |
| 24 | Resin A(20) | C-26 | 3/7 | KF96* | 40 |

"Resin A" of Tables 9 to 11 means a resin A1 having a structural unit represented by the formula (A-1) and a structural unit represented by the formula (B), or a resin A2 having a structural unit represented by the formula (A-2) and a structural unit represented by the formula (B). "Resin C" of Tables 9 to 11 means a resin C having a structural unit represented by the formula (C). "Resin A/resin C mixing ratio" of Tables 9 to 11 means a mixing ratio (in a mass ratio) of a resin A and a resin C. "Compound D" of Tables 9 to 11 means a compound D having structural units represented by the formulas (O-1) and (O-2), or KF96. "Mass% of compound D to resin A" of Tables 9 to 11 means the ratio in % by mass of a compound D contained in each charge-transporting layer to the total mass of a resin A1 and a resin A2 contained in the charge-transporting layer.

**(Table 12)**

| Example | Potential variation (\/) | Initial torque relative value | Torque relative value after making 5000 copies | Number average particle size (nm) |
|---|---|---|---|---|
| 1 | 35 | 0.74 | 0.77 | 460 |
| 2 | 41 | 0.64 | 0.68 | 530 |
| 3 | 47 | 0.55 | 0.59 | 670 |
| 4 | 52 | 0.53 | 0.56 | 750 |
| 5 | 37 | 0.72 | 0.74 | 470 |
| 6 | 53 | 0.52 | 0.57 | 820 |
| 7 | 38 | 0.74 | 0.77 | 490 |
| 8 | 54 | 0.55 | 0.57 | 830 |
| 9 | 35 | 0.74 | 0.77 | 450 |
| 10 | 53 | 0.53 | 0.56 | 740 |
| 11 | 36 | 0.73 | 0.75 | 430 |
| 12 | 54 | 0.53 | 0.53 | 800 |
| 13 | 37 | 0.72 | 0.77 | 470 |
| 14 | 53 | 0.53 | 0.54 | 820 |
| 15 | 38 | 0.74 | 0.75 | 490 |
| 16 | 54 | 0.54 | 0.59 | 800 |
| 17 | 37 | 0.74 | 0.8 | 450 |
| 18 | 55 | 0.53 | 0.57 | 740 |
| 19 | 38 | 0.73 | 0.79 | 430 |
| 20 | 54 | 0.52 | 0.55 | 800 |
| 21 | 44 | 0.62 | 0.66 | 540 |
| 22 | 46 | 0.57 | 0.62 | 640 |
| 23 | 44 | 0.63 | 0.68 | 530 |
| 24 | 49 | 0.59 | 0.64 | 660 |
| 25 | 43 | 0.62 | 0.66 | 520 |
| 26 | 46 | 0.57 | 0.62 | 640 |
| 27 | 44 | 0.63 | 0.68 | 580 |
| 28 | 47 | 0.59 | 0.64 | 680 |
| 29 | 49 | 0.59 | 0.64 | 630 |
| 30 | 43 | 0.62 | 0.66 | 170 |
| 31 | 44 | 0.63 | 0.68 | 960 |
| 32 | 47 | 0.73 | 0.77 | 1630 |
| 33 | 37 | 0.72 | 0.74 | 220 |
| 34 | 49 | 0.59 | 0.64 | 660 |
| 35 | 45 | 0.62 | 0.66 | 540 |
| 36 | 46 | 0.57 | 0.62 | 1230 |
| 37 | 47 | 0.59 | 0.64 | 690 |
| 38 | 37 | 0.73 | 0.77 | 360 |
| 39 | 37 | 0.73 | 0.77 | 310 |
| 40 | 47 | 0.56 | 0.64 | 760 |
| 41 | 46 | 0.57 | 0.62 | 720 |
| 42 | 49 | 0.59 | 0.64 | 690 |
| 43 | 48 | 0.58 | 0.63 | 680 |
| 44 | 49 | 0.59 | 0.64 | 650 |
| 45 | 45 | 0.62 | 0.66 | 960 |
| 46 | 47 | 0.74 | 0.8 | 530 |
| 47 | 46 | 0.57 | 0.62 | 1020 |
| 48 | 56 | 0.55 | 0.6 | 1210 |

**(Table 13)**

| Example | Potential variation (V) | Initial torque relative value | Torque relative value after making 5000 copies | Number average particle size (nm) |
|---|---|---|---|---|
| 49 | 46 | 0.73 | 0.77 | 460 |
| 50 | 52 | 0.63 | 0.68 | 530 |
| 51 | 58 | 0.56 | 0.59 | 670 |
| 52 | 63 | 0.52 | 0.56 | 750 |
| 53 | 48 | 0.72 | 0.74 | 470 |
| 54 | 64 | 0.52 | 0.57 | 820 |
| 55 | 49 | 0.74 | 0.77 | 490 |
| 56 | 65 | 0.55 | 0.57 | 800 |
| 57 | 46 | 0.74 | 0.77 | 450 |
| 58 | 64 | 0.53 | 0.56 | 740 |
| 59 | 47 | 0.73 | 0.75 | 430 |
| 60 | 65 | 0.52 | 0.53 | 800 |
| 61 | 48 | 0.72 | 0.77 | 470 |
| 62 | 64 | 0.52 | 0.54 | 820 |
| 63 | 39 | 0.74 | 0.75 | 490 |
| 64 | 55 | 0.55 | 0.6 | 800 |
| 65 | 38 | 0.74 | 0.8 | 450 |
| 66 | 56 | 0.53 | 0.57 | 740 |
| 67 | 39 | 0.73 | 0.79 | 430 |
| 68 | 76 | 0.52 | 0.55 | 800 |
| 69 | 64 | 0.52 | 0.54 | 820 |
| 70 | 69 | 0.57 | 0.62 | 950 |
| 71 | 73 | 0.52 | 0.54 | 1640 |
| 72 | 57 | 0.57 | 0.62 | 640 |
| 73 | 53 | 0.63 | 0.68 | 530 |
| 74 | 58 | 0.59 | 0.64 | 660 |
| 75 | 54 | 0.62 | 0.66 | 520 |
| 76 | 57 | 0.57 | 0.62 | 640 |
| 77 | 53 | 0.63 | 0.68 | 580 |
| 78 | 58 | 0.59 | 0.64 | 660 |
| 79 | 44 | 0.62 | 0.66 | 520 |
| 80 | 47 | 0.57 | 0.62 | 640 |
| 81 | 38 | 0.72 | 0.74 | 470 |
| 82 | 46 | 0.52 | 0.56 | 750 |
| 83 | 47 | 0.72 | 0.74 | 470 |
| 84 | 48 | 0.52 | 0.56 | 750 |
| 85 | 66 | 0.52 | 0.55 | 1060 |
| 86 | 69 | 0.57 | 0.62 | 950 |
| 87 | 73 | 0.52 | 0.54 | 1640 |
| 88 | 73 | 0.52 | 0.54 | 1440 |
| 89 | 44 | 0.62 | 0.66 | 170 |
| 90 | 44 | 0.62 | 0.66 | 540 |
| 91 | 47 | 0.57 | 0.62 | 640 |
| 92 | 49 | 0.57 | 0.62 | 950 |
| 93 | 47 | 0.57 | 0.62 | 640 |
| 94 | 44 | 0.62 | 0.66 | 540 |
| 95 | 58 | 0.59 | 0.64 | 660 |

**(Table 14)**

| Comparative Example | Potential variation (V) | Initial torque relative value | Torque relative value after making 5000 copies | Number average particle size (nm) |
|---|---|---|---|---|
| 1 | 26 | 1.00 | 1.00 | No domains formed |
| 2 | 121 | 0.33 | 1.02 | No domains formed |
| 3 | 118 | 0.46 | 1.00 | No domains formed |
| 4 | 113 | 0.53 | 1.12 | No domains formed |
| 5 | 147 | 0.35 | 1.06 | No domains formed |
| 6 | 135 | 0.45 | 0.99 | No domains formed |
| 7 | 155 | 0.57 | 1.04 | No domains formed |
| 8 | 169 | 0.54 | 1.13 | No domains formed |
| 9 | 175 | 0.53 | 1.05 | No domains formed |
| 10 | 179 | 0.46 | 1.02 | No domains formed |
| 11 | 177 | 0.52 | 1.00 | No domains formed |
| 12 | 157 | 0.4 | 0.98 | No domains formed |
| 13 | 166 | 0.52 | 1.12 | No domains formed |
| 14 | 168 | 0.5 | 1.03 | No domains formed |
| 15 | 170 | 0.48 | 1.04 | No domains formed |
| 16 | 173 | 0.44 | 1.02 | No domains formed |
| 17 | 178 | 0.47 | 1.14 | No domains formed |
| 18 | 173 | 0.43 | 1.02 | No domains formed |
| 19 | 126 | 0.56 | 0.79 | 460 |
| 20 | 179 | 0.48 | 0.78 | 470 |
| 21 | 122 | 0.52 | 0.77 | 680 |
| 22 | 170 | 0.47 | 0.79 | 530 |
| 23 | 127 | 0.52 | 0.75 | 480 |
| 24 | 169 | 0.45 | 0.77 | 650 |

Based on comparison between Examples and Comparative Examples 1 to 18, the effect of persistently relaxing the contact stress cannot be attained in each of Comparative Examples because the charge-transporting layer contains neither the resin A1 nor the resin A2. This is revealed because torque is not sufficiently reduced in the evaluation performed as described above at the initial stage and after outputting 5,000 copies.

On the other hand, since domains containing the resin A1, the resin A2 and the compound D are formed in a matrix containing the resin C in each of Examples, torque is excellently reduced in the evaluation performed after outputting 5,000 copies, and thus, the effect of persistently relaxing the contact stress is exhibited.

Based on comparison between Examples and Comparative Examples 2 to 18, since the charge-transporting layer contains neither the resin A1 nor the resin A2 in each of Comparative Examples, the effect of suppressing potential variation cannot be sufficiently exhibited. Besides, since domains are not formed, it is suggested that the compound D has moved to the surface of the electrophotographic photosensitive member and the interface with the charge-generating layer because the charge-transporting layer contains neither the resin A1 nor the resin A2 in each of Comparative Examples. It is presumed that the compound D having moved to the interface with the charge-generating layer forms a barrier to charge movement, and hence the potential variation cannot be sufficiently reduced.

On the other hand, since domains containing the resin A1, the resin A2 and the compound D are formed in a matrix containing the resin C in each of Examples, the effect of suppressing potential variation is excellently exhibited. It is presumed that movement of the compound D to the interface with the charge-generating layer can be suppressed by forming the domains containing the resin A1, the resin A2 and the compound D, and as a result, the potential variation is suppressed.

Based on comparison between Examples and Comparative Examples 19 to 24, although the effect of persistently relaxing the contact stress can be exhibited in these comparative examples, the potential variation is large. Furthermore, a matrix-domain structure is found in these comparative examples. Accordingly, it is suggested that KF96 does not remain within domains although KF96 forms a matrix-domain structure together with the resin A1, the resin A2 and the resin C. It is probably because KF96 does not have a structure of the compound D of the present invention, affinity with the resin A is so low that KF96 has moved to the surface and the interface with the charge-generating layer.

Based on these results, it seems that excellent effects of persistently relaxing the contact stress and suppressing the potential variation can be exhibited because the affinity between the compound D and the resins A1 and A2 is so high that the compound D can remain within the domains.

While the present invention has been described with reference to exemplary embodiments, it is to be understood that the invention is not limited to the disclosed exemplary embodiments. The scope of the following claims is to be accorded the broadest interpretation so as to encompass all such modifications and equivalent structures and functions.

A charge-transporting layer of an electrophotographic photosensitive member contains a charge-transporting substance, a resin A having a specific structural unit and a resin C having a specific structural unit as resins, and a compound D having a specific structural unit, and the charge-transporting layer contains domains containing the resin A1, the resin A2 and the compound D in a matrix containing the charge-transporting substance and the resin C.

## Claims

1. An electrophotographic photosensitive member comprising:
a support;
a charge-generating layer formed on the support; and
a charge-transporting layer formed on the charge-generating layer;
wherein the charge-transporting layer is a surface layer of the electrophotographic photosensitive member, and
the charge-transporting layer has a matrix-domain structure having:
a domain which comprises:
a compound D having a structural unit represented by the following formula (0-1) and a structural unit represented by the following formula (0-2); and
at least one resin selected from the group consisting of:
a resin A1 having a structural unit represented by the following formula (A-1) and a structural unit represented by the following formula (B), and
a resin A2 having a structural unit represented by the following formula (A-2) and a structural unit represented by the following formula (B); and
a matrix which comprises:
a resin C having a structural unit represented by the following formula (C); and
a charge-transporting substance;
wherein
a content of the structural unit represented by the formula (A-1) and the structural unit represented by the formula (A-2) is from 10% by mass to 40% by mass based on the total mass of the resin A1 and the resin A2, where,
m¹¹ represents 0 or 1,
X¹¹ represents an ortho-phenylene group, a metaphenylene group, a para-phenylene group, a bivalent group having two para-phenylene groups bonded with a methylene group, or a bivalent group having two para-phenylene groups bonded with an oxygen atom,
Z¹¹ and Z¹² each independently represents an alkylene group having 1 to 4 carbon atoms,
R¹¹ to R¹⁴ each independently represents an alkyl group having 1 to 4 carbon atoms, or a phenyl group, and
n¹¹ represents the repetition number of a structure within brackets, and an average of n¹¹ in the resin A1 ranges from 20 to 150,
where,
m²¹ represents 0 or 1,
X²¹ represents an ortho-phenylene group, a metaphenylene group, a para-phenylene group, a bivalent group having two para-phenylene groups bonded with a methylene group, or a bivalent group having two para-phenylene groups bonded with an oxygen atom,
Z²¹ to Z²³ each independently represents an alkylene group having 1 to 4 carbon atoms,
R¹⁶ to R²⁷ each independently represents an alkyl group having 1 to 4 carbon atoms, or a phenyl group, and
n²¹, n²² and n²³ each independently represents the repetition number of a structure within brackets, an average of n²¹ in the resin A2 ranges from 1 to 10, an average of n²² in the resin A2 ranges from 1 to 10, and an average of n²³ in the resin A2 ranges from 20 to 200,
where,
m³¹ represents 0 or 1,
X³¹ represents an ortho-phenylene group, a metaphenylene group, a para-phenylene group, a bivalent group having two para-phenylene groups bonded with a methylene group, or a bivalent group having two para-phenylene groups bonded with an oxygen atom,
Y³¹ represents a single bond, a methylene group, an ethylidene group, a propylidene group, a cyclohexylidene group, a phenylmethylene group, a phenylethylidene group or an oxygen atom, and
R³¹ to R³⁸ each independently represents a hydrogen atom or a methyl group,
where,
m⁴¹ represents 0 or 1,
X⁴¹ represents an ortho-phenylene group, a metaphenylene group, a para-phenylene group, a bivalent group having two para-phenylene groups bonded with a methylene group, or a bivalent group having two para-phenylene groups bonded with an oxygen atom,
Y⁴¹ represents a single bond, a methylene group, an ethylidene group, a propylidene group, a cyclohexylidene group, a phenylmethylene group, a phenylethylidene group or an oxygen atom, and
R⁴¹ to R⁴⁸ each independently represents a hydrogen atom or a methyl group,
where,
R⁶¹ represents a hydrogen atom or a methyl group,
R⁶² represents a phenyl group, a cyano group, a carbamoyl group, or a group represented by the formula - COOR⁶⁴, where R⁶⁴ represents a hydrogen atom, a methyl group, an ethyl group, a propyl group, an isopropyl group, a butyl group, an isobutyl group, a 2-ethylhexyl group, a nonyl group, an isononyl group, a cyclohexyl group, a 2-methoxyethyl group or a 2-hydroxyethyl group,
R⁶³ represents a hydrogen atom or a methyl group, and
n⁶¹ represents the repetition number of a structure within brackets, and an average of n⁶¹ in the compound D ranges from 1 to 500.

2. The electrophotographic photosensitive member according to claim 1, wherein a content of the compound D in the charge-transporting layer is from 1% by mass to 50% by mass based on the total mass of the resin A1 and the resin A2.

3. The electrophotographic photosensitive member according to claim 1 or 2, wherein R⁶² represents a phenyl group or a group represented by the formula -COOR⁶⁴, where R⁶⁴ represents a hydrogen atom, a methyl group, a 2-ethylhexyl group, a 2-methoxyethyl group or a 2-hydroxyethyl group.

4. The electrophotographic photosensitive member according to any one of claims 1 to 3, wherein a content of the compound D is from 0.1% by mass to 20% by mass based on a total mass of all resins contained in the charge-transporting layer.

5. The electrophotographic photosensitive member according to any one of claims 1 to 4, wherein the charge-transporting substance is at least one selected from the group consisting of a triarylamine compound, a hydrazone compound, a butadiene compound and an enamine compound.

6. The electrophotographic photosensitive member according to any one of claims 1 to 5, wherein a content of the charge-transporting substance is from 25% by mass to 70% by mass based on a total mass of the charge-transporting layer.

7. The electrophotographic photosensitive member according to any one of claims 1 to 6, wherein a total content of the resin A1 and the resin A2 is from 5% by mass to 50% by mass based on a total mass of all resins contained in the charge-transporting layer.

8. A method for producing an electrophotographic photosensitive member comprising a support, a charge-generating layer formed on the support, and a charge-transporting layer formed on the charge-generating layer, the charge-transporting layer being a surface layer of the electrophotographic photosensitive member, the method comprising:
preparing a charge-transporting layer coating solution containing:
at least one resin selected from the group consisting of:
a resin A1 having a structural unit represented by the following formula (A-1) and a structural unit represented by the following formula (B); and
a resin A2 having a structural unit represented by the following formula (A-2) and a structural unit represented by the following formula (B);
a compound D having a structural unit represented by the following formula (O-1) and a structural unit represented by the following formula (0-2);
a resin C having a structural unit represented by the following formula (C); and
a charge-transporting substance; and
forming the charge-transporting layer by forming a coating film of the charge-transporting layer coating solution and drying the coating film,
wherein a content of the structural unit represented by the formula (A-1) and the structural unit represented by the formula (A-2) is from 10% by mass to 40% by mass based on a total mass of the resin A1 and the resin A2,
where,
m¹¹ represents 0 or 1,
X¹¹ represents an ortho-phenylene group, a metaphenylene group, a para-phenylene group, a bivalent group having two para-phenylene groups bonded with a methylene group, or a bivalent group having two para-phenylene groups bonded with an oxygen atom,
Z¹¹ and Z¹² each independently represents an alkylene group having 1 to 4 carbon atoms,
R¹¹ to R¹⁴ each independently represents an alkyl group having 1 to 4 carbon atoms, or a phenyl group, and
n¹¹ represents the repetition number of a structure within brackets, and an average of n¹¹ in the resin A1 ranges from 20 to 150,
where,
m²¹ represents 0 or 1,
X²¹ represents an ortho-phenylene group, a metaphenylene group, a para-phenylene group, a bivalent group having two para-phenylene groups bonded with a methylene group, or a bivalent group having two para-phenylene groups bonded with an oxygen atom,
Z²¹ to Z²³ each independently represents an alkylene group having 1 to 4 carbon atoms,
R¹⁶ to R²⁷ each independently represents an alkyl group having 1 to 4 carbon atoms, or a phenyl group, and
n²¹, n²² and n²³ each independently represents the repetition number of a structure within brackets, an average of n²¹ in the resin A2 ranges from 1 to 10, an average of n²² in the resin A2 ranges from 1 to 10, and an average of n²³ in the resin A2 ranges from 20 to 200,
where,
m³¹ represents 0 or 1,
X³¹ represents an ortho-phenylene group, a metaphenylene group, a para-phenylene group, a bivalent group having two para-phenylene groups bonded with a methylene group, or a bivalent group having two para-phenylene groups bonded with an oxygen atom,
Y³¹ represents a single bond, a methylene group, an ethylidene group, a propylidene group, a cyclohexylidene group, a phenylmethylene group, a phenylethylidene group or an oxygen atom, and
R³¹ to R³⁸ each independently represents a hydrogen atom or a methyl group,
where,
m⁴¹ represents 0 or 1,
X⁴¹ represents an ortho-phenylene group, a metaphenylene group, a para-phenylene group, a bivalent group having two para-phenylene groups bonded with a methylene group, or a bivalent group having two para-phenylene groups bonded with an oxygen atom,
Y⁴¹ represents a single bond, a methylene group, an ethylidene group, a propylidene group, a cyclohexylidene group, a phenylmethylene group, a phenylethylidene group or an oxygen atom, and
R⁴¹ to R⁴⁸ each independently represents a hydrogen atom or a methyl group,
where,
R⁶¹ represents a hydrogen atom or a methyl group,
R⁶² represents a phenyl group, a cyano group, a carbamoyl group, or a group represented by the formula - COOR⁶⁴, where R⁶⁴ represents a hydrogen atom, a methyl group, an ethyl group, a propyl group, an isopropyl group, a butyl group, an isobutyl group, a 2-ethylhexyl group, a nonyl group, an isononyl group, a cyclohexyl group, a 2-methoxyethyl group or a 2-hydroxyethyl group,
R⁶³ represents a hydrogen atom or a methyl group, and
n⁶¹ represents the repetition number of a structure within brackets, and an average of n⁶¹ in the compound D ranges from 1 to 500.

9. A process cartridge detachably attachable to a main body of an electrophotographic apparatus, wherein the process cartridge integrally supports:
the electrophotographic photosensitive member according to any one of claims 1 to 7, and
at least one device selected from the group consisting of a charging device, a developing device, a transferring device and a cleaning device.

10. An electrophotographic apparatus comprising:
the electrophotographic photosensitive member according to any one of claims 1 to 7; and
a charging device, an exposing device, a developing device and a transferring device.

## Patentansprüche

1. Elektrophotographisches photosensitives Element, das umfasst:
einen Träger;
eine Ladungs-erzeugende Schicht, die auf dem Träger gebildet ist;
und eine Ladungs-transportierende Schicht, die auf der Ladungserzeugenden Schicht gebildet ist;
wobei die Ladungs-transportierende Schicht eine Oberflächenschicht des elektrophotographischen photosensitiven Elements ist, und
die Ladungs-transportierende Schicht eine Matrix-Domänen-Struktur aufweist, die aufweist:
eine Domäne, welche umfasst:
eine Verbindung D mit einer durch die folgende Formel (O-1) dargestellten Struktureinheit und einer durch die folgende Formel (O-2) dargestellten Struktureinheit; und
zumindest ein Harz ausgewählt aus der Gruppe bestehend aus:
einem Harz A1 mit einer durch die folgenden Formel (A-1) dargestellten Struktureinheit und einer durch die folgende Formel (B) dargestellten Struktureinheit, und
einem Harz A2 mit einer durch die folgende Formel (A-2) dargestellten Struktureinheit und einer durch die folgende Formel (B) dargestellten Struktureinheit; und
eine Matrix, welche umfasst:
ein Harz C mit einer durch die folgende Formel (C) dargestellten Struktureinheit; und
eine Ladungs-transportierende Substanz;
wobei
ein Gehalt der durch die Formel (A-1) dargestellten Struktureinheit und der durch die Formel (A-2) dargestellten Struktureinheit von 10 Massen-% bis 40 Massen-% basierend auf der Gesamtmasse des Harzes A1 und des Harzes A2 ist,
wobei,
m¹¹ 0 oder 1 darstellt,
X¹¹ eine ortho-Phenylengruppe, eine meta-Phenylengruppe, eine para-Phenylengruppe, eine bivalente Gruppe mit zwei para-Phenylengruppen, die mit einer Methylengruppe verbunden sind, oder eine bivalente Gruppe mit zwei para-Phenylengruppen, die mit einem Sauerstoffatom verbunden sind, darstellt,
Z¹¹ und Z¹² jeweils unabhängig eine Alkylengruppe mit 1 bis 4 Kohlenstoffatomen darstellen,
R¹¹ bis R¹⁴ jeweils unabhängig eine Alkylgruppe mit 1 bis 4 Kohlenstoffatomen oder eine Phenylgruppe darstellen, und
n¹¹ eine Wiederholungsanzahl einer Struktur in den Klammern darstellt und ein Mittelwert von n¹¹ in dem Harz A1 von 20 bis 150 reicht,
wobei,
m²¹ 0 oder 1 darstellt,
X²¹ eine ortho-Phenylengruppe, eine meta-Phenylengruppe, eine para-Phenylengruppe, eine bivalente Gruppe mit zwei para-Phenylengruppen, die mit einer Methylengruppe verbunden sind, oder eine bivalente Gruppe mit zwei para-Phenylengruppen, die mit einem Sauerstoffatom verbunden sind, darstellt,
Z²¹ bis Z²³ jeweils unabhängig eine Alkylengruppe mit 1 bis 4 Kohlenstoffatomen darstellen,
R¹⁶ bis R²⁷ jeweils unabhängig eine Alkylgruppe mit 1 bis 4 Kohlenstoffatomen oder eine Phenylgruppe darstellen, und
n²¹, n²² und n²³ jeweils unabhängig die Wiederholungsanzahl einer Struktur in den Klammern darstellen, ein Mittelwert von n²¹ in dem Harz A2 von 1 bis 10 reicht, ein Mittelwert von n²² in dem Harz A2 von 1 bis 10 reicht, und ein Mittelwert von n²³ in dem Harz A2 von 20 bis 200 reicht,
wobei
m³¹ 0 oder 1 darstellt,
X³¹ eine ortho-Phenylengruppe, eine meta-Phenylengruppe, eine para-Phenylengruppe, eine bivalente Gruppe mit zwei para-Phenylengruppen, die mit einer Methylengruppe verbunden sind, oder eine bivalente Gruppe mit zwei para-Phenylengruppen, die mit einem Sauerstoffatom verbunden sind, darstellt,
Y³¹ eine Einfachbindung, eine Methylengruppe, eine Ethylidengruppe, eine Propylidengruppe, eine Cyclohexylidengruppe, eine Phenylmethylengruppe, eine Phenylethylidengruppe oder ein Sauerstoffatom darstellt, und
R³¹ bis R³⁸ jeweils unabhängig ein Wasserstoffatom oder eine Methylgruppe darstellen,
wobei,
m⁴¹ 0 oder 1 darstellt,
X⁴¹ eine ortho-Phenylengruppe, eine meta-Phenylengruppe, eine para-Phenylengruppe, eine bivalente Gruppe mit zwei para-Phenylengruppen, die mit einer Methylengruppe verbunden sind, oder eine bivalente Gruppe mit zwei para-Phenylengruppen, die mit einem Sauerstoffatom verbunden sind, darstellt,
Y⁴¹ eine Einfachbindung, eine Methylengruppe, eine Ethylidengruppe, eine Propylidengruppe, eine Cyclohexylidengruppe, eine Phenylmethylengruppe, eine Phenylethylidengruppe oder ein Sauerstoffatom darstellt, und
R⁴¹ bis R⁴⁸ jeweils unabhängig ein Wasserstoffatom oder eine Methylgruppe darstellen,
wobei,
R⁶¹ ein Wasserstoffatom oder eine Methylgruppe darstellt,
R⁶² eine Phenylgruppe, eine Cyanogruppe, eine Carbamoylgruppe oder eine durch die Formel -COOR⁶⁴ dargestellte Gruppe darstellt, wobei R⁶⁴ ein Wasserstoffatom, eine Methylgruppe, eine Ethylgruppe, eine Propylgruppe, eine Isopropylgruppe, eine Butylgruppe, eine Isobutylgruppe, eine 2-Ethylhexylgruppe, eine Nonylgruppe, eine Isononylgruppe, eine Cyclohexylgruppe, eine 2-Methoxyethylgruppe oder eine 2-Hydroxyethylgruppe darstellt,
R⁶³ ein Wasserstoffatom oder eine Methylgruppe darstellt, und
n⁶¹ eine Wiederholungsanzahl einer Struktur in den Klammern darstellt und ein Mittelwert von n⁶¹ in der Verbindung D von 1 bis 500 reicht.

2. Elektrophotographisches photosensitives Element nach Anspruch 1, wobei ein Gehalt der Verbindung D in der Ladungs-transportierenden Schicht von 1 Massen-% bis 50 Massen-% basierend auf der Gesamtmasse des Harzes A1 und des Harzes A2 ist.

3. Elektrophotographisches photosensitives Element nach Anspruch 1 oder 2, wobei R⁶² eine Phenylgruppe oder eine durch die Formel -COOR⁶⁴ dargestellte Gruppe darstellt, wobei R⁶⁴ ein Wasserstoffatom, eine Methylgruppe, eine 2-Ethylhexylgruppe, eine 2-Methoxyethylgruppe oder eine 2-Hydroxyethylgruppe darstellt.

4. Elektrophotographisches photosensitives Element nach einem der Ansprüche 1 bis 3, wobei ein Gehalt der Verbindung D von 0,1 Massen-% bis 20 Massen-% basierend auf der Gesamtmasse aller in der Ladungs-transportierenden Schicht enthaltenen Harze ist.

5. Elektrophotographisches photosensitives Element nach einem der Ansprüche 1 bis 4, wobei die Ladungs-transportierende Substanz zumindest Eine ist, die aus der Gruppe ausgewählt ist, die aus einer Triarylaminverbindung, einer Hydrazonverbindung, einer Butadienverbindung und einer Enaminverbindung besteht.

6. Elektrophotographisches photosensitives Element nach einem der Ansprüche 1 bis 5, wobei ein Gehalt der Ladungs-transportierenden Substanz von 25 Massen-% bis 70 Massen-% basierend auf der Gesamtmasse der Ladungs-transportierenden Schicht ist.

7. Elektrophotographisches photosensitives Element nach einem der Ansprüche 1 bis 6, wobei ein Gesamtgehalt des Harzes A1 und des Harzes A2 von 5 Massen-% bis 50 Massen-% basierend auf einer Gesamtmasse aller in der Ladungs-transportierenden Schicht enthaltenen Harze ist.

8. Verfahren zum Herstellen eines elektrophotographischen photosensitiven Elements, das einen Träger, eine Ladungs-erzeugende Schicht, die auf dem Träger gebildet ist, und eine Ladungs-transportierende Schicht, die auf der Ladungs-erzeugenden Schicht gebildet ist, umfasst, wobei die Ladungs-transportierende Schicht eine Oberflächenschicht des elektrophotographischen photosensitiven Elements ist, wobei das Verfahren umfasst:
Anfertigen einer Ladungs-transportierende-Schicht-Beschichtungslösung, die enthält:
zumindest ein Harz ausgewählt aus der Gruppe bestehend aus:
einem Harz Al mit einer durch die folgende Formel (A-1) dargestellten Struktureinheit und einer durch die folgende Formel (B) dargestellten Struktureinheit; und
einem Harz A2 mit einer durch die folgende Formel (A-2) dargestellten Struktureinheit und einer durch die folgende Formel (B) dargestellten Struktureinheit;
eine Verbindung D mit einer durch die folgende Formel (O-1) dargestellten Struktureinheit und einer durch die folgende Formel (O-2) dargestellten Struktureinheit;
ein Harz C mit einer durch die folgende Formel (C) dargestellten Struktureinheit; und
eine Ladungs-transportierende Substanz; und
Bilden der Ladungs-transportierenden Schicht durch Bilden eines Beschichtungsfilms aus der Ladungs-transportierende-Schicht-Beschichtungslösung und Trocknen des Beschichtungsfilms,
wobei ein Gehalt der durch die Formel (A-1) dargestellten Struktureinheit und der durch die Formel (A-2) dargestellten Struktureinheit von 10 Massen-% bis 40 Massen-% basierend auf einer Gesamtmasse des Harzes A1 und des Harzes A2 ist,
wobei,
m¹¹ 0 oder 1 darstellt,
X¹¹ eine ortho-Phenylengruppe, eine meta-Phenylengruppe, eine para-Phenylengruppe, eine bivalente Gruppe mit zwei para-Phenylengruppen, die mit einer Methylengruppe verbunden sind, oder eine bivalente Gruppe mit zwei para-Phenylengruppen, die mit einem Sauerstoffatom verbunden sind, darstellt,
Z¹¹ und Z¹² jeweils unabhängig eine Alkylengruppe mit 1 bis 4 Kohlenstoffatomen darstellen,
R¹¹ bis R¹⁴ jeweils unabhängig eine Alkylgruppe mit 1 bis 4 Kohlenstoffatomen oder eine Phenylgruppe darstellen, und
n¹¹ eine Wiederholungsanzahl einer Struktur in den Klammern darstellt und ein Mittelwert von n¹¹ in dem Harz A1 von 20 bis 150 reicht,
wobei,
m²¹ 0 oder 1 darstellt,
X²¹ eine ortho-Phenylengruppe, eine meta-Phenylengruppe, eine para-Phenylengruppe, eine bivalente Gruppe mit zwei para-Phenylengruppen, die mit einer Methylengruppe verbunden sind, oder eine bivalente Gruppe mit zwei para-Phenylengruppen, die mit einem Sauerstoffatom verbunden sind, darstellt,
Z²¹ bis Z²³ jeweils unabhängig eine Alkylengruppe mit 1 bis 4 Kohlenstoffatomen darstellen,
R¹⁶ bis R²⁷ jeweils unabhängig eine Alkylgruppe mit 1 bis 4 Kohlenstoffatomen oder eine Phenylgruppe darstellen, und
n²¹, n²² und n²³ jeweils unabhängig die Wiederholungsanzahl einer Struktur in den Klammern darstellt, ein Mittelwert von n²¹ in dem Harz A2 von 1 bis 10 reicht, ein Mittelwert von n²² in dem Harz A2 von 1 bis 10 reicht, und ein Mittelwert von n²³ in dem Harz A2 von 20 bis 200 reicht,
wobei
m³¹ 0 oder 1 darstellt,
X³¹ eine ortho-Phenylengruppe, eine meta-Phenylengruppe, eine para-Phenylengruppe, eine bivalente Gruppe mit zwei para-Phenylengruppen, die mit einer Methylengruppe verbunden sind, oder eine bivalente Gruppe mit zwei para-Phenylengruppen, die mit einem Sauerstoffatom verbunden sind, darstellt,
Y³¹ eine Einfachbindung, eine Methylengruppe, eine Ethylidengruppe, eine Propylidengruppe, eine Cyclohexylidengruppe, eine Phenylmethylengruppe, eine Phenylethylidengruppe oder ein Sauerstoffatom darstellt, und
R³¹ bis R³⁸ jeweils unabhängig ein Wasserstoffatom oder eine Methylgruppe darstellen,
wobei,
m⁴¹ 0 oder 1 darstellt,
X⁴¹ eine ortho-Phenylengruppe, eine meta-Phenylengruppe, eine para-Phenylengruppe, eine bivalente Gruppe mit zwei para-Phenylengruppen, die mit einer Methylengruppe verbunden sind, oder eine bivalente Gruppe mit zwei para-Phenylengruppen, die mit einem Sauerstoffatom verbunden sind, darstellt,
Y⁴¹ eine Einfachbindung, eine Methylengruppe, eine Ethylidengruppe, eine Propylidengruppe, eine Cyclohexylidengruppe, eine Phenylmethylengruppe, eine Phenylethylidengruppe oder ein Sauerstoffatom darstellt, und
R⁴¹ bis R⁴⁸ jeweils unabhängig ein Wasserstoffatom oder eine Methylgruppe darstellen.
wobei
R⁶¹ ein Wasserstoffatom oder eine Methylgruppe darstellt,
R⁶² eine Phenylgruppe, eine Cyanogruppe, eine Carbamoylgruppe oder eine durch die Formel -COOR⁶⁴ dargestellte Gruppe darstellt, wobei R⁶⁴ ein Wasserstoffatom, eine Methylgruppe, eine Ethylgruppe, eine Propylgruppe, eine Isopropylgruppe, eine Butylgruppe, eine Isobutylgruppe, eine 2-Ethylhexylgruppe, eine Nonylgruppe, eine Isononylgruppe, eine Cyclohexylgruppe, eine 2-Methoxyethylgruppe oder eine 2-Hydroxyethylgruppe darstellt,
R⁶³ ein Wasserstoffatom oder eine Methylgruppe darstellt, und
n⁶¹ eine Wiederholungsanzahl einer Struktur in den Klammern darstellt und ein Mittelwert von n⁶¹ in der Verbindung D von 1 bis 500 reicht.

9. Prozesskartusche, die abnehmbar zu einem Hauptkörper eines elektrophotographischen Apparats montierbar ist, wobei die Prozesskartusche integral trägt:
das elektrophotographische photosensitive Element nach einem der Ansprüche 1 bis 7, und
zumindest eine Vorrichtung, die aus der Gruppe ausgewählt ist, die aus einer Ladungsvorrichtung, einer Entwicklungsvorrichtung, einer Transfervorrichtung und einer Reinigungsvorrichtung besteht.

10. Elektrophotographischer Apparat, der umfasst:
das elektrophotographische photosensitive Element nach einem der Ansprüche 1 bis 7; und
eine Ladungsvorrichtung, eine Belichtungsvorrichtung, eine Entwicklungsvorrichtung und eine Transfervorrichtung.

## Revendications

1. Elément photosensible électrophotographique comprenant :
un support ;
une couche de production de charge formée sur le support ; et
une couche de transport de charge formée sur la couche de production de charge ;
dans lequel la couche de transport de charge est une couche de surface de l'élément photosensible électrophotographique, et
la couche de transport de charge comporte une structure de matrice-domaine comportant :
un domaine qui comprend :
un composé D ayant un motif structural représenté par la formule (O-1) suivante et un motif structural représenté par la formule (O-2) suivante ; et
au moins une résine choisie dans le groupe consistant en :
une résine A1 ayant un motif structural représenté par la formule (A-1) suivante et un motif structural représenté par la formule (B) suivante, et
une résine A2 ayant un motif structural représenté par la formule (A-2) suivante et un motif structural représenté par la formule (B) suivante ; et
une matrice qui comprend :
une résine C ayant un motif structural représenté par la formule (C) suivante ; et
une substance de transport de charge ;
où :
la quantité du motif structural représenté par la formule (A-1) et du motif structural représenté par la formule (A-2) va de 10 % en masse à 40 % en masse sur la base de la masse totale de la résine Al et de la résine A2,
où
m¹¹ est égal à 0 ou 1,
X¹¹ représente un groupe ortho-phénylène, un groupe méta-phénylène, un groupe para-phénylène, un groupe bivalent comportant deux groupes para-phénylène liés avec un groupe méthylène, ou un groupe bivalent comportant deux groupes para-phénylène liés avec un atome d'oxygène,
Z¹¹ et Z¹² représentent chacun indépendamment un groupe alkylène ayant 1 à 4 atomes de carbone,
R¹¹ à R¹⁴ représentent chacun indépendamment un groupe alkyle ayant 1 à 4 atomes de carbone, ou un groupe phényle, et
n¹¹ représente le nombre de répétitions d'une structure entre crochets, et la moyenne de n¹¹ dans la résine A1 va de 20 à 150,
où
m²¹ est égal à 0 ou 1,
X²¹ représente un groupe ortho-phénylène, un groupe méta-phénylène, un groupe para-phénylène, un groupe bivalent ayant deux groupes para-phénylène liés avec un groupe méthylène, ou un groupe bivalent ayant deux groupes para-phénylène liés avec un atome d'oxygène,
Z²¹ à Z²³ représentent chacun indépendamment un groupe alkylène ayant 1 à 4 atomes de carbone,
R¹⁶ à R²⁷ représentent chacun indépendamment un groupe alkyle ayant 1 à 4 atomes de carbone, ou un groupe phényle, et
n²¹ n²², et n²³ représentent chacun indépendamment le nombre de répétitions d'une structure entre crochets, la moyenne de n²¹ dans la résine A2 va de 1 à 10, la moyenne de n²² dans la résine A2 va de 1 à 10 et la moyenne de n²³ dans la résine A2 va de 20 à 200,
où
m³¹ est égal à 0 ou 1,
X³¹ représente un groupe ortho-phénylène, un groupe méta-phénylène, un groupe para-phénylène, un groupe bivalent ayant deux groupes para-phénylène liés avec un groupe méthylène, ou un groupe bivalent ayant deux groupes para-phénylène liés avec un atome d'oxygène,
Y³¹ représente une liaison simple, un groupe méthylène, un groupe éthylidène, un groupe propylidène, un groupe cyclohexylidène, un groupe phénylméthylène, un groupe phényléthylidène ou un atome d'oxygène,
R³¹ à R³⁸ représentent chacun indépendamment un atome d'hydrogène ou un groupe méthyle,
Où
m⁴¹ est égal à 0 ou 1,
X⁴¹ représente un groupe ortho-phénylène, un groupe méta-phénylène, un groupe para-phénylène, un groupe bivalent ayant deux groupes para-phénylène liés avec un groupe méthylène, ou un groupe bivalent ayant deux groupes para-phénylène liés avec un atome d'oxygène,
Y⁴¹ représente une liaison simple, un groupe méthylène, un groupe éthylidène, un groupe propylidène, un groupe cyclohexylidène, un groupe phénylméthylène, un groupe phényléthylidène ou un atome d'oxygène, et
R⁴¹ à R⁴⁸ représentent chacun indépendamment un atome d'hydrogène ou un groupe méthyle,
où
R⁶¹ représente un atome d'hydrogène ou un groupe méthyle,
R⁶² représente un groupe phényle, un groupe cyano, un groupe carbamoyle, ou un groupe représenté par la formule -COOR⁶⁴, dans laquelle R⁶⁴ représente un atome d'hydrogène, un groupe méthyle, un groupe éthyle, un groupe propyle, un groupe isopropyle, un groupe butyle, un groupe isobutyle, un groupe 2-éthylhexyle, un groupe nonyle, un groupe isononyle, un groupe cyclohexyle, un groupe 2-méthoxyéthyle ou un groupe 2-hydroxyéthyle,
R⁶³ représente un atome d'hydrogène ou un groupe méthyle, et
n⁶¹ représente le nombre de répétitions d'une structure entre crochets, et la moyenne de n⁶¹ dans le composé D va de 1 à 500.

2. Elément photosensible électrophotographique suivant la revendication 1, dans lequel la quantité du composé D dans la couche de transport de charge va de 1 % en masse à 50 % en masse sur la base de la masse totale de la résine A1 et de la résine A2.

3. Elément photosensible électrophotographique suivant la revendication 1 ou 2, dans lequel R⁶² représente un groupe phényle ou un groupe représenté par la formule -COOR⁶⁴, dans laquelle R⁶⁴ représente un atome d'hydrogène, un groupe méthyle, un groupe 2-éthylhexyle, un groupe 2-méthoxyéthyle ou un groupe 2-hydroxyéthyle,

4. Elément photosensible électrophotographique suivant l'une quelconque des revendications 1 à 3, dans lequel la quantité du composé D va de 0,1 % en masse à 20 % en masse sur la base de la masse totale de toutes les résines présentes dans la couche de transport de charge.

5. Elément photosensible électrophotographique suivant l'une quelconque des revendications 1 à 4, dans lequel la substance de transport de charge est au moins une substance choisie dans le groupe consistant en un dérivé de triarylamine, un dérivé d'hydrazone, un dérivé de butadiène et un dérivé d'énamine.

6. Elément photosensible électrophotographique suivant l'une quelconque des revendications 1 à 5, dans lequel la quantité de la substance de transport de charge va de 25 % en masse à 70 % en masse sur la base de la masse totale de la couche de transport de charge.

7. Elément photosensible électrophotographique suivant l'une quelconque des revendications 1 à 6, dans lequel la quantité totale de la résine A1 et de la résine A2 va de 5 % en masse à 50 % en masse sur la base de la masse totale de toutes les résines présentes dans la couche de transport de charge.

8. Procédé pour la production d'un élément photosensible électrophotographique comprenant un support, une couche de production de charge formée sur le support, une couche de transport de charge formée sur la couche de production de charge, la couche de transport de charge étant une couche de surface de l'élément photosensible électrophotographique, le procédé comprenant :
la préparation d'une solution de revêtement de formation de couche de transport de charge contenant :
au moins une résine choisie dans le groupe consistant en :
une résine A1 ayant un motif structural représenté par la formule (A-1) suivante et un motif structural représenté par la formule (B) suivante ; et
une résine A2 ayant un motif structural représenté par la formule (A-2) suivante et un motif structural représenté par la formule (B) suivante ;
un composé D ayant un motif structural représenté par la formule (O-1) suivante et un motif structural représenté par la formule (O-2) suivante ;
une résine (C) ayant un motif structural représenté par la formule (C) suivante ; et
une substance de transport de charge ; et
la formation de la couche de transport de charge en formant un film de revêtement de la solution de revêtement de formation de couche de transport de charge et en séchant le film de revêtement,
où la quantité du motif structural représenté par la formule (A-1) et du motif structural représenté par la formule (A-2) va de 10 % en masse à 40 % en masse sur la base de la masse totale de la résine A1 et de la résine A2,
où
m¹¹ est égal à 0 ou 1,
X¹¹ représente un groupe ortho-phénylène, un groupe méta-phénylène, un groupe para-phénylène, un groupe bivalent ayant deux groupes para-phénylène liés avec un groupe méthylène, ou un groupe bivalent ayant deux groupes para-phénylène liés avec un atome d'oxygène,
Z¹¹ et Z¹² représentent chacun indépendamment un groupe alkylène ayant 1 à 4 atomes de carbone,
R¹¹ à R¹⁴ représentent chacun indépendamment un groupe alkyle ayant 1 à 4 atomes de carbone, ou un groupe phényle, et
n¹¹ représente le nombre de répétitions d'une structure entre crochets, et la moyenne de n¹¹ dans la résine A1 va de 20 à 150,
où
m²¹ est égal à 0 ou 1,
X²¹ représente un groupe ortho-phénylène, un groupe méta-phénylène, un groupe para-phénylène, un groupe bivalent ayant deux groupes para-phénylène liés avec un groupe méthylène, ou un groupe bivalent ayant deux groupes para-phénylène liés avec un atome d'oxygène,
Z²¹ à Z²³ représentent chacun indépendamment un groupe alkylène ayant 1 à 4 atomes de carbone,
R¹⁶ à R²⁷ représentent chacun indépendamment un groupe alkyle ayant 1 à 4 atomes de carbone, ou un groupe phényle, et
n²¹ n²², et n²³ représentent chacun indépendamment le nombre de répétitions d'une structure entre crochets, la moyenne de n²¹ dans la résine A2 va de 1 à 10, la moyenne de n²² dans la résine A2 va de 1 à 10 et la moyenne de n²³ dans la résine A2 va de 20 à 200,
m³¹ est égal à 0 ou 1,
X³¹ représente un groupe ortho-phénylène, un groupe méta-phénylène, un groupe para-phénylène, un groupe bivalent ayant deux groupes para-phénylène liés avec un groupe méthylène, ou un groupe bivalent ayant deux groupes para-phénylène liés avec un atome d'oxygène,
Y³¹ représente une liaison simple, un groupe méthylène, un groupe éthylidène, un groupe propylidène, un groupe cyclohexylidène, un groupe phénylméthylène, un groupe phényléthylidène ou un atome d'oxygène, et
R³¹ à R³⁸ représentent chacun indépendamment un atome d'hydrogène ou un groupe méthyle,
où m⁴¹ est égal à 0 ou 1,
X⁴¹ représente un groupe ortho-phénylène, un groupe méta-phénylène, un groupe para-phénylène, un groupe bivalent ayant deux groupes para-phénylène liés avec un groupe méthylène, ou un groupe bivalent ayant deux groupes para-phénylène liés avec un atome d'oxygène,
Y⁴¹ représente une liaison simple, un groupe méthylène, un groupe éthylidène, un groupe propylidène, un groupe cyclohexylidène, un groupe phénylméthylène, un groupe phényléthylidène ou un atome d'oxygène, et
R⁴¹ à R⁴⁸ représentent chacun indépendamment un atome d'hydrogène ou un groupe méthyle,
où
R⁶¹ représente un atome d'hydrogène ou un groupe méthyle,
R⁶² représente un groupe phényle, un groupe cyano, un groupe carbamoyle, ou un groupe représenté par la formule -COOR⁶⁴, dans laquelle R⁶⁴ représente un atome d'hydrogène, un groupe méthyle, un groupe éthyle, un groupe propyle, un groupe isopropyle, un groupe butyle, un groupe isobutyle, un groupe 2-éthylhexyle, un groupe nonyle, un groupe isononyle, un groupe cyclohexyle, un groupe 2-méthoxyéthyle ou un groupe 2-hydroxyéthyle,
R⁶³ représente un atome d'hydrogène ou un groupe méthyle, et
n⁶¹ représente le nombre de répétitions d'une structure entre crochets, et la moyenne de n⁶¹ dans le composé D va de 1 à 500.

9. Cartouche de traitement pouvant être fixée de manière amovible au corps principal d'un appareil électrophotographique, ladite cartouche de traitement portant de manière intégrée :
l'élément photosensible électrophotographique suivant l'une quelconque des revendications 1 à 7, et
au moins un dispositif choisi dans le groupe consistant en un dispositif de charge, un dispositif de développement, un dispositif de transfert, un dispositif de nettoyage.

10. Appareil électrophotographique comprenant :
l'élément photosensible électrophotographique suivant l'une quelconque des revendications 1 à 7 ; et
un dispositif de charge et un dispositif d'exposition, un dispositif de développement et un dispositif de transfert.
